



US011898223B2

(12) **United States Patent**  
Sherman et al.

(10) **Patent No.:** US 11,898,223 B2  
(45) **Date of Patent:** \*Feb. 13, 2024

(54) **DEGRADABLE METAL MATRIX COMPOSITE**

(71) Applicant: **Terves Inc.**, Euclid, OH (US)

(72) Inventors: **Andrew J. Sherman**, Mentor, OH (US); **Nicholas Farkas**, Euclid, OH (US); **David Wolf**, Euclid, OH (US)

(73) Assignee: **Terves, LLC**, Euclid, OH (US)

(\*) Notice: Subject to any disclaimer, the term of this patent is extended or adjusted under 35 U.S.C. 154(b) by 586 days.

This patent is subject to a terminal disclaimer.

(21) Appl. No.: **17/018,547**

(22) Filed: **Sep. 11, 2020**

(65) **Prior Publication Data**

US 2020/0407822 A1 Dec. 31, 2020

**Related U.S. Application Data**

(63) Continuation of application No. 16/045,924, filed on Jul. 26, 2018.

(Continued)

(51) **Int. Cl.**

**C22C 1/10** (2023.01)  
**C22C 29/02** (2006.01)

(Continued)

(52) **U.S. Cl.**

CPC ..... **C22C 1/1068** (2013.01); **C22C 1/047** (2023.01); **C22C 1/101** (2013.01); **C22C 1/1036** (2013.01); **C22C 21/00** (2013.01); **C22C 23/00** (2013.01); **C22C 29/02** (2013.01); **C22C 29/06** (2013.01); **C22C 29/12** (2013.01); **C22C 29/14** (2013.01); **C22C 29/16** (2013.01); **C22C 29/18** (2013.01); **C22C 32/0036**

(2013.01); **C22C 32/0052** (2013.01); **C22C 32/0057** (2013.01); **C22C 32/0063** (2013.01); **C22C 32/0068** (2013.01);

(Continued)

(58) **Field of Classification Search**

CPC ..... C22C 1/1068  
See application file for complete search history.

(56)

**References Cited**

U.S. PATENT DOCUMENTS

1,468,905 A 7/1923 Herman  
1,558,066 A 10/1925 Veazey et al.

(Continued)

FOREIGN PATENT DOCUMENTS

CA 2783241 6/2011  
CA 2783346 6/2011

(Continued)

OTHER PUBLICATIONS

Scharf et al., "Corrosion of AX 91 Secondary Magnesium Alloy", Advanced Engineering Materials, vol. 7, No. 12, pp. 1134-1142 (2005).

(Continued)

*Primary Examiner* — Christopher S Kessler

(74) *Attorney, Agent, or Firm* — Ulmer & Berne LLP;  
Brian E. Turung

(57)

**ABSTRACT**

The present invention relates to the composition and production of an engineered degradable metal matrix composite that is useful in constructing temporary systems requiring wear resistance, high hardness, and/or high resistance to deformation in water-bearing applications such as, but not limited to, oil and gas completion operations.

**13 Claims, 6 Drawing Sheets**



## Related U.S. Application Data

|      |                                                                                                                                                                                            |             |         |                       |
|------|--------------------------------------------------------------------------------------------------------------------------------------------------------------------------------------------|-------------|---------|-----------------------|
| (60) | Provisional application No. 62/537,707, filed on Jul. 27, 2017.                                                                                                                            | 3,660,049 A | 5/1972  | Benjamin              |
|      |                                                                                                                                                                                            | 3,765,484 A | 10/1973 | Hamby, Jr. et al.     |
|      |                                                                                                                                                                                            | 3,768,563 A | 10/1973 | Blount                |
|      |                                                                                                                                                                                            | 3,775,823 A | 12/1973 | Adolph et al.         |
|      |                                                                                                                                                                                            | 3,816,080 A | 6/1974  | Bomford et al.        |
|      |                                                                                                                                                                                            | 3,823,045 A | 7/1974  | Hielema               |
|      |                                                                                                                                                                                            | 3,878,889 A | 4/1975  | Seabourne             |
|      |                                                                                                                                                                                            | 3,894,850 A | 7/1975  | Kovalchuk et al.      |
|      |                                                                                                                                                                                            | 3,924,677 A | 12/1975 | Prenner et al.        |
| (51) | <b>Int. Cl.</b>                                                                                                                                                                            | 3,957,483 A | 5/1976  | Suzuki                |
|      | <i>C22C 47/04</i> (2006.01)                                                                                                                                                                | 4,010,583 A | 3/1977  | Highberg              |
|      | <i>C22C 32/00</i> (2006.01)                                                                                                                                                                | 4,039,717 A | 8/1977  | Titus                 |
|      | <i>C22C 23/00</i> (2006.01)                                                                                                                                                                | 4,050,529 A | 9/1977  | Tagirov et al.        |
|      | <i>C22C 21/00</i> (2006.01)                                                                                                                                                                | 4,157,732 A | 6/1979  | Fonner                |
|      | <i>C22C 29/06</i> (2006.01)                                                                                                                                                                | 4,248,307 A | 2/1981  | Silberman et al.      |
|      | <i>C22C 29/18</i> (2006.01)                                                                                                                                                                | 4,264,362 A | 4/1981  | Serveg et al.         |
|      | <i>C22C 49/04</i> (2006.01)                                                                                                                                                                | 4,284,137 A | 8/1981  | Taylor                |
|      | <i>C22C 29/16</i> (2006.01)                                                                                                                                                                | 4,292,377 A | 9/1981  | Petersen et al.       |
|      | <i>C22C 47/12</i> (2006.01)                                                                                                                                                                | 4,368,788 A | 1/1983  | Drake                 |
|      | <i>C22C 29/14</i> (2006.01)                                                                                                                                                                | 4,372,384 A | 2/1983  | Kinney                |
|      | <i>C22C 29/12</i> (2006.01)                                                                                                                                                                | 4,373,584 A | 2/1983  | Silberman et al.      |
|      | <i>C22C 1/047</i> (2023.01)                                                                                                                                                                | 4,373,952 A | 2/1983  | Parent                |
| (52) | <b>U.S. Cl.</b>                                                                                                                                                                            | 4,374,543 A | 2/1983  | Richardson            |
|      | CPC ..... <i>C22C 32/0073</i> (2013.01); <i>C22C 32/0078</i> (2013.01); <i>C22C 47/04</i> (2013.01); <i>C22C 47/12</i> (2013.01); <i>C22C 49/04</i> (2013.01); <i>C22C 1/047</i> (2023.01) | 4,384,616 A | 5/1983  | Dellinger             |
|      |                                                                                                                                                                                            | 4,395,440 A | 7/1983  | Abe et al.            |
|      |                                                                                                                                                                                            | 4,399,871 A | 8/1983  | Adkins et al.         |
|      |                                                                                                                                                                                            | 4,407,368 A | 10/1983 | Erbstoesser           |
|      |                                                                                                                                                                                            | 4,422,508 A | 12/1983 | Rutledge, Jr. et al.  |
|      |                                                                                                                                                                                            | 4,450,136 A | 5/1984  | Dudek et al.          |
|      |                                                                                                                                                                                            | 4,452,311 A | 6/1984  | Speegle et al.        |
|      |                                                                                                                                                                                            | 4,475,729 A | 10/1984 | Costigan              |
|      |                                                                                                                                                                                            | 4,498,543 A | 2/1985  | Pye et al.            |
|      |                                                                                                                                                                                            | 4,499,048 A | 2/1985  | Hanejko               |
|      |                                                                                                                                                                                            | 4,499,049 A | 2/1985  | Hanejko               |
|      |                                                                                                                                                                                            | 4,524,825 A | 6/1985  | Fore                  |
|      |                                                                                                                                                                                            | 4,526,840 A | 7/1985  | Jerabek               |
|      |                                                                                                                                                                                            | 4,534,414 A | 8/1985  | Pringle               |
|      |                                                                                                                                                                                            | 4,539,175 A | 9/1985  | Lichti et al.         |
|      |                                                                                                                                                                                            | 4,554,986 A | 11/1985 | Jones                 |
|      |                                                                                                                                                                                            | 4,619,699 A | 10/1986 | Petkovic-Luton et al. |
|      |                                                                                                                                                                                            | 4,640,354 A | 2/1987  | Boisson               |
|      |                                                                                                                                                                                            | 4,648,901 A | 3/1987  | Murray et al.         |
|      |                                                                                                                                                                                            | 4,655,852 A | 4/1987  | Rallis                |
|      |                                                                                                                                                                                            | 4,664,962 A | 5/1987  | DesMarais, Jr.        |
|      |                                                                                                                                                                                            | 4,668,470 A | 5/1987  | Gilman et al.         |
|      |                                                                                                                                                                                            | 4,673,549 A | 6/1987  | Ecer                  |
|      |                                                                                                                                                                                            | 4,674,572 A | 6/1987  | Gallus                |
|      |                                                                                                                                                                                            | 4,678,037 A | 7/1987  | Smith                 |
|      |                                                                                                                                                                                            | 4,681,133 A | 7/1987  | Weston                |
|      |                                                                                                                                                                                            | 4,688,641 A | 8/1987  | Knieriemen            |
|      |                                                                                                                                                                                            | 4,690,796 A | 9/1987  | Paliwal               |
|      |                                                                                                                                                                                            | 4,693,863 A | 9/1987  | Del Corso et al.      |
|      |                                                                                                                                                                                            | 4,703,807 A | 11/1987 | Weston                |
|      |                                                                                                                                                                                            | 4,706,753 A | 11/1987 | Ohkochi et al.        |
|      |                                                                                                                                                                                            | 4,708,202 A | 11/1987 | Sukup et al.          |
|      |                                                                                                                                                                                            | 4,708,208 A | 11/1987 | Halbardier            |
|      |                                                                                                                                                                                            | 4,709,761 A | 12/1987 | Setterberg, Jr.       |
|      |                                                                                                                                                                                            | 4,714,116 A | 12/1987 | Brunner               |
|      |                                                                                                                                                                                            | 4,716,964 A | 1/1988  | Erbstoesser et al.    |
|      |                                                                                                                                                                                            | 4,719,971 A | 1/1988  | Owens                 |
|      |                                                                                                                                                                                            | 4,721,159 A | 1/1988  | Ohkochi et al.        |
|      |                                                                                                                                                                                            | 4,738,599 A | 4/1988  | Shilling              |
|      |                                                                                                                                                                                            | 4,741,973 A | 5/1988  | Condit et al.         |
|      |                                                                                                                                                                                            | 4,768,588 A | 9/1988  | Kupsa                 |
|      |                                                                                                                                                                                            | 4,775,598 A | 10/1988 | Jaeckel               |
|      |                                                                                                                                                                                            | 4,784,226 A | 11/1988 | Wyatt                 |
|      |                                                                                                                                                                                            | 4,805,699 A | 2/1989  | Halbardier            |
|      |                                                                                                                                                                                            | 4,817,725 A | 4/1989  | Jenkins               |
|      |                                                                                                                                                                                            | 4,834,184 A | 5/1989  | Streich et al.        |
|      |                                                                                                                                                                                            | H635 H      | 6/1989  | Johnson et al.        |
|      |                                                                                                                                                                                            | 4,853,056 A | 8/1989  | Hoffman               |
|      |                                                                                                                                                                                            | 4,869,324 A | 9/1989  | Holder                |
|      |                                                                                                                                                                                            | 4,869,325 A | 9/1989  | Halbardier            |
|      |                                                                                                                                                                                            | 4,875,948 A | 10/1989 | Vernecker             |
|      |                                                                                                                                                                                            | 4,880,059 A | 11/1989 | Brandell et al.       |
|      |                                                                                                                                                                                            | 4,889,187 A | 12/1989 | Terrell et al.        |
|      |                                                                                                                                                                                            | 4,890,675 A | 1/1990  | Dew                   |
|      |                                                                                                                                                                                            | 4,901,794 A | 2/1990  | Baugh et al.          |
|      |                                                                                                                                                                                            | 4,909,320 A | 3/1990  | Hebert et al.         |

## References Cited

## U.S. PATENT DOCUMENTS

|             |         |                      |
|-------------|---------|----------------------|
| 1,880,614 A | 10/1932 | Wetherill et al.     |
| 2,352,993 A | 7/1933  | Albertson            |
| 2,011,613 A | 8/1935  | Brown et al.         |
| 2,094,578 A | 10/1937 | Blumenthal et al.    |
| 2,189,697 A | 2/1940  | Baker                |
| 2,222,233 A | 11/1940 | Mize                 |
| 2,225,143 A | 12/1940 | Baker et al.         |
| 2,238,895 A | 4/1941  | Gage                 |
| 2,261,292 A | 11/1941 | Salnikov             |
| 2,294,648 A | 9/1942  | Ansel et al.         |
| 2,301,624 A | 11/1942 | Holt                 |
| 2,394,843 A | 2/1946  | Cook et al.          |
| 2,672,199 A | 3/1954  | McKenna              |
| 2,753,941 A | 7/1956  | Hebard et al.        |
| 2,754,910 A | 7/1956  | Derrick et al.       |
| 2,933,136 A | 4/1960  | Ayers et al.         |
| 2,983,634 A | 5/1961  | Budininkas et al.    |
| 3,057,405 A | 10/1962 | Mallinger            |
| 3,066,391 A | 12/1962 | Vordahl et al.       |
| 3,106,959 A | 10/1963 | Huitt et al.         |
| 3,142,338 A | 7/1964  | Brown                |
| 3,152,009 A | 10/1964 | DeLong               |
| 3,180,728 A | 4/1965  | Pryor et al.         |
| 3,180,778 A | 4/1965  | Rinderspacher et al. |
| 3,196,949 A | 7/1965  | Thomas               |
| 3,226,314 A | 12/1965 | Wellington et al.    |
| 3,242,988 A | 3/1966  | McGuire, Jr. et al.  |
| 3,295,935 A | 1/1967  | Pflumm et al.        |
| 3,298,440 A | 1/1967  | Current              |
| 3,316,748 A | 5/1967  | Lang et al.          |
| 3,326,291 A | 6/1967  | Zandemer             |
| 3,347,714 A | 10/1967 | Broverman et al.     |
| 3,385,696 A | 5/1968  | Hitchcock et al.     |
| 3,390,724 A | 7/1968  | Caldwell             |
| 3,395,758 A | 8/1968  | Kelly et al.         |
| 3,406,101 A | 10/1968 | Kilpatrick           |
| 3,416,918 A | 12/1968 | Roberts              |
| 3,434,539 A | 3/1969  | Merritt              |
| 3,445,148 A | 5/1969  | Harris et al.        |
| 3,445,731 A | 5/1969  | Saeki et al.         |
| 3,465,181 A | 9/1969  | Colby et al.         |
| 3,489,218 A | 1/1970  | Means                |
| 3,513,230 A | 5/1970  | Rhees et al.         |
| 3,600,163 A | 8/1971  | Badia et al.         |
| 3,602,305 A | 8/1971  | Kisling              |
| 3,637,446 A | 1/1972  | Elliott et al.       |
| 3,645,331 A | 2/1972  | Maurer et al.        |

(56)

## References Cited

## U.S. PATENT DOCUMENTS

|             |         |                       |             |         |                    |
|-------------|---------|-----------------------|-------------|---------|--------------------|
| 4,916,029 A | 4/1990  | Nagle et al.          | 5,417,285 A | 5/1995  | Van Buskirk et al. |
| 4,917,966 A | 4/1990  | Wilde et al.          | 5,425,424 A | 6/1995  | Reinhardt et al.   |
| 4,921,664 A | 5/1990  | Couper                | 5,427,177 A | 6/1995  | Jordan, Jr. et al. |
| 4,929,415 A | 5/1990  | Okazaki               | 5,435,392 A | 7/1995  | Kennedy            |
| 4,932,474 A | 6/1990  | Schroeder, Jr. et al. | 5,439,051 A | 8/1995  | Kennedy et al.     |
| 4,934,459 A | 6/1990  | Baugh et al.          | 5,454,430 A | 10/1995 | Kennedy et al.     |
| 4,938,309 A | 7/1990  | Emdy                  | 5,456,317 A | 10/1995 | Hood, III et al.   |
| 4,938,809 A | 7/1990  | Das et al.            | 5,456,327 A | 10/1995 | Denton et al.      |
| 4,944,351 A | 7/1990  | Eriksen et al.        | 5,464,062 A | 11/1995 | Blizzard, Jr.      |
| 4,949,788 A | 8/1990  | Szarka et al.         | 5,472,048 A | 12/1995 | Kennedy            |
| 4,952,902 A | 8/1990  | Kawaguchi et al.      | 5,474,131 A | 12/1995 | Jordan, Jr. et al. |
| 4,975,412 A | 12/1990 | Okazaki et al.        | 5,476,632 A | 12/1995 | Shivanath et al.   |
| 4,977,958 A | 12/1990 | Miller                | 5,477,923 A | 12/1995 | Jordan, Jr. et al. |
| 4,981,177 A | 1/1991  | Carmody et al.        | 5,479,986 A | 1/1996  | Gano et al.        |
| 4,986,361 A | 1/1991  | Mueller et al.        | 5,494,538 A | 2/1996  | Kirillov et al.    |
| 4,997,622 A | 3/1991  | Regazzoni et al.      | 5,506,055 A | 4/1996  | Dorfman et al.     |
| 5,006,044 A | 4/1991  | Walker, Sr. et al.    | 5,507,439 A | 4/1996  | Story              |
| 5,010,955 A | 4/1991  | Springer              | 5,511,620 A | 4/1996  | Baugh et al.       |
| 5,036,921 A | 8/1991  | Pittard et al.        | 5,524,699 A | 6/1996  | Cook               |
| 5,048,611 A | 9/1991  | Cochran               | 5,526,880 A | 6/1996  | Jordan, Jr. et al. |
| 5,049,165 A | 9/1991  | Tslesin               | 5,526,881 A | 6/1996  | Martin et al.      |
| 5,061,323 A | 10/1991 | DeLucchia             | 5,529,746 A | 6/1996  | Knoss et al.       |
| 5,063,775 A | 11/1991 | Walker, Sr. et al.    | 5,531,735 A | 7/1996  | Thompson           |
| 5,073,207 A | 12/1991 | Faure et al.          | 5,533,573 A | 7/1996  | Jordan, Jr. et al. |
| 5,074,361 A | 12/1991 | Brisco et al.         | 5,536,485 A | 7/1996  | Kume et al.        |
| 5,076,869 A | 12/1991 | Bourell et al.        | 5,552,110 A | 9/1996  | Iba                |
| 5,084,088 A | 1/1992  | Okazaki               | 5,558,153 A | 9/1996  | Holcombe et al.    |
| 5,087,304 A | 2/1992  | Chang et al.          | 5,601,924 A | 2/1997  | Beane et al.       |
| 5,090,480 A | 2/1992  | Pittard et al.        | 5,607,017 A | 3/1997  | Owens et al.       |
| 5,095,988 A | 3/1992  | Bode                  | 5,623,993 A | 4/1997  | Van Buskirk et al. |
| 5,103,911 A | 4/1992  | Heijnen               | 5,623,994 A | 4/1997  | Robinson           |
| 5,106,702 A | 4/1992  | Walker et al.         | 5,641,023 A | 6/1997  | Ross et al.        |
| 5,117,915 A | 6/1992  | Mueller et al.        | 5,636,691 A | 7/1997  | Hendrickson et al. |
| 5,143,795 A | 9/1992  | Das et al.            | 5,647,444 A | 7/1997  | Williams           |
| 5,161,614 A | 11/1992 | Wu et al.             | 5,665,289 A | 9/1997  | Chung et al.       |
| 5,171,734 A | 12/1992 | Sanjurjo et al.       | 5,677,372 A | 10/1997 | Yamamoto et al.    |
| 5,178,216 A | 1/1993  | Giroux et al.         | 5,685,372 A | 11/1997 | Gano               |
| 5,181,571 A | 1/1993  | Mueller et al.        | 5,701,576 A | 12/1997 | Fujita et al.      |
| 5,183,631 A | 2/1993  | Kugimiya et al.       | 5,707,214 A | 1/1998  | Schmidt            |
| 5,188,182 A | 2/1993  | Echols, III et al.    | 5,709,269 A | 1/1998  | Head               |
| 5,188,183 A | 2/1993  | Hopmann et al.        | 5,720,344 A | 2/1998  | Newman             |
| 5,204,055 A | 4/1993  | Sachs et al.          | 5,722,033 A | 2/1998  | Carden             |
| 5,222,867 A | 6/1993  | Walker, Sr. et al.    | 5,728,195 A | 3/1998  | Eastman et al.     |
| 5,226,483 A | 7/1993  | Williamson, Jr.       | 5,765,639 A | 6/1998  | Muth               |
| 5,228,518 A | 7/1993  | Wilson et al.         | 5,767,562 A | 6/1998  | Yamashita          |
| 5,234,055 A | 8/1993  | Cornette              | 5,772,735 A | 6/1998  | Sehgal et al.      |
| 5,238,646 A | 8/1993  | Tarcy et al.          | 5,782,305 A | 7/1998  | Hicks              |
| 5,240,495 A | 8/1993  | Dieckmann et al.      | 5,797,454 A | 8/1998  | Hipp               |
| 5,240,742 A | 8/1993  | Johnson et al.        | 5,820,608 A | 10/1998 | Luzio et al.       |
| 5,252,365 A | 10/1993 | White                 | 5,826,652 A | 10/1998 | Tapp               |
| 5,253,714 A | 10/1993 | Davis et al.          | 5,826,661 A | 10/1998 | Parker et al.      |
| 5,271,468 A | 12/1993 | Streich et al.        | 5,829,520 A | 11/1998 | Johnson            |
| 5,273,569 A | 12/1993 | Gilman et al.         | 5,836,396 A | 11/1998 | Norman             |
| 5,282,509 A | 2/1994  | Schurr, III           | 5,857,521 A | 1/1999  | Ross et al.        |
| 5,285,798 A | 2/1994  | Banerjee et al.       | 5,881,816 A | 3/1999  | Wright             |
| 5,292,478 A | 3/1994  | Scorey                | 5,896,819 A | 4/1999  | Turila et al.      |
| 5,293,940 A | 3/1994  | Hromas et al.         | 5,902,424 A | 5/1999  | Fujita et al.      |
| 5,304,260 A | 4/1994  | Aikawa et al.         | 5,934,372 A | 8/1999  | Muth               |
| 5,304,588 A | 4/1994  | Boysen et al.         | 5,941,309 A | 8/1999  | Appleton           |
| 5,309,874 A | 5/1994  | Willermet et al.      | 5,960,881 A | 10/1999 | Allamont et al.    |
| 5,310,000 A | 5/1994  | Arterbury et al.      | 5,964,965 A | 10/1999 | Schulz et al.      |
| 5,316,598 A | 5/1994  | Chang et al.          | 5,894,007 A | 11/1999 | Yuan et al.        |
| 5,318,746 A | 6/1994  | Lashmore et al.       | 5,980,602 A | 11/1999 | Carden             |
| 5,336,466 A | 8/1994  | Iba                   | 5,985,466 A | 11/1999 | Atarashi et al.    |
| 5,342,576 A | 8/1994  | Whitehead             | 5,988,287 A | 11/1999 | Jordan, Jr. et al. |
| 5,352,522 A | 10/1994 | Kugimiya et al.       | 5,990,051 A | 11/1999 | Ischy et al.       |
| 5,380,473 A | 1/1995  | Bogue et al.          | 5,992,452 A | 11/1999 | Nelson, II         |
| 5,387,380 A | 2/1995  | Cima et al.           | 5,992,520 A | 11/1999 | Schultz et al.     |
| 5,392,860 A | 2/1995  | Ross                  | 6,007,314 A | 12/1999 | Nelson, II         |
| 5,394,236 A | 2/1995  | Murnick               | 6,024,915 A | 2/2000  | Kume et al.        |
| 5,394,941 A | 3/1995  | Venditto et al.       | 6,030,637 A | 2/2000  | Whitehead          |
| 5,398,754 A | 3/1995  | Dinhoble              | 6,032,735 A | 3/2000  | Echols             |
| 5,407,011 A | 4/1995  | Layton                | 6,033,622 A | 3/2000  | Maruyama           |
| 5,409,555 A | 4/1995  | Fujita et al.         | 6,036,777 A | 3/2000  | Sachs              |
| 5,411,082 A | 5/1995  | Kennedy               | 6,040,087 A | 3/2000  | Chu et al.         |
|             |         |                       | 6,047,773 A | 4/2000  | Kawakami           |
|             |         |                       | 6,050,340 A | 4/2000  | Zeltmann et al.    |
|             |         |                       | 6,069,313 A | 5/2000  | Scott              |
|             |         |                       |             |         | Kay                |

(56)

## References Cited

## U.S. PATENT DOCUMENTS

|              |         |                    |              |         |                      |
|--------------|---------|--------------------|--------------|---------|----------------------|
| 6,076,600 A  | 6/2000  | Vick, Jr. et al.   | 6,591,915 B2 | 7/2003  | Burris et al.        |
| 6,079,496 A  | 6/2000  | Hirth              | 6,601,648 B2 | 8/2003  | Ebinger              |
| 6,085,837 A  | 7/2000  | Massinon et al.    | 6,601,650 B2 | 8/2003  | Sundararajan         |
| 6,095,247 A  | 8/2000  | Streich et al.     | 6,609,569 B2 | 8/2003  | Towlett et al.       |
| 6,119,783 A  | 9/2000  | Parker et al.      | 6,612,826 B1 | 9/2003  | Bauer et al.         |
| 6,126,898 A  | 10/2000 | Butler             | 6,613,383 B1 | 9/2003  | George et al.        |
| 6,142,237 A  | 11/2000 | Christmas et al.   | 6,619,400 B2 | 9/2003  | Brumet               |
| 6,161,622 A  | 12/2000 | Robb et al.        | 6,630,008 B1 | 10/2003 | Meeks, III et al.    |
| 6,167,970 B1 | 1/2001  | Stout et al.       | 6,634,428 B2 | 10/2003 | Krauss et al.        |
| 6,170,583 B1 | 1/2001  | Boyce              | 6,662,886 B2 | 12/2003 | Russell              |
| 6,171,359 B1 | 1/2001  | Levinski et al.    | 6,675,889 B1 | 1/2004  | Mullins et al.       |
| 6,173,779 B1 | 1/2001  | Smith              | 6,699,305 B2 | 3/2004  | Myrick               |
| 6,176,323 B1 | 1/2001  | Weirich et al.     | 6,712,153 B2 | 3/2004  | Turley et al.        |
| 6,189,616 B1 | 2/2001  | Gano et al.        | 6,712,797 B1 | 3/2004  | Southern, Jr.        |
| 6,189,618 B1 | 2/2001  | Beeman et al.      | 6,713,177 B2 | 3/2004  | George et al.        |
| 6,213,202 B1 | 4/2001  | Read, Jr.          | 6,715,541 B2 | 4/2004  | Pedersen et al.      |
| 6,220,349 B1 | 4/2001  | Vargas et al.      | 6,737,385 B2 | 5/2004  | Todd et al.          |
| 6,220,350 B1 | 4/2001  | Brothers et al.    | 6,779,599 B2 | 8/2004  | Mullins et al.       |
| 6,220,357 B1 | 4/2001  | Carmichael et al.  | 6,799,638 B2 | 10/2004 | Butterfield, Jr.     |
| 6,228,904 B1 | 5/2001  | Yadav et al.       | 6,810,960 B2 | 11/2004 | Pia                  |
| 6,230,799 B1 | 5/2001  | Slaughter et al.   | 6,817,414 B2 | 11/2004 | Lee                  |
| 6,237,688 B1 | 5/2001  | Burleson et al.    | 6,831,044 B2 | 12/2004 | Constien             |
| 6,238,280 B1 | 5/2001  | Ritt et al.        | 6,883,611 B2 | 4/2005  | Smith et al.         |
| 6,241,021 B1 | 6/2001  | Bowling            | 6,887,297 B2 | 5/2005  | Winter et al.        |
| 6,248,399 B1 | 6/2001  | Hehmann            | 6,896,049 B2 | 5/2005  | Moyes                |
| 6,250,392 B1 | 6/2001  | Muth               | 6,896,061 B2 | 5/2005  | Hriscu et al.        |
| 6,261,432 B1 | 7/2001  | Huber et al.       | 6,899,777 B2 | 5/2005  | Vaidyanathan et al.  |
| 6,265,205 B1 | 7/2001  | Hitchens et al.    | 6,908,516 B2 | 6/2005  | Hehmann et al.       |
| 6,273,187 B1 | 8/2001  | Voisin, Jr. et al. | 6,913,827 B2 | 7/2005  | Georget et al.       |
| 6,276,452 B1 | 8/2001  | Davis et al.       | 6,926,086 B2 | 8/2005  | Patterson et al.     |
| 6,276,457 B1 | 8/2001  | Moffatt et al.     | 6,932,159 B2 | 8/2005  | Hovem                |
| 6,279,656 B1 | 8/2001  | Sinclair et al.    | 6,939,388 B2 | 9/2005  | Angelius             |
| 6,287,332 B1 | 9/2001  | Bolz et al.        | 6,945,331 B2 | 9/2005  | Patel                |
| 6,287,445 B1 | 9/2001  | Lashmore et al.    | 6,951,331 B2 | 10/2005 | Haughom et al.       |
| 6,302,205 B1 | 10/2001 | Ryll               | 6,959,759 B2 | 11/2005 | Doane et al.         |
| 6,315,041 B1 | 11/2001 | Carlisle et al.    | 6,973,970 B2 | 12/2005 | Johnston et al.      |
| 6,315,050 B2 | 11/2001 | Vaylnsheyn et al.  | 6,973,973 B2 | 12/2005 | Howard et al.        |
| 6,325,148 B1 | 12/2001 | Trahan et al.      | 6,983,796 B2 | 1/2006  | Bayne et al.         |
| 6,328,110 B1 | 12/2001 | Joubert            | 6,986,390 B2 | 1/2006  | Doane et al.         |
| 6,341,653 B1 | 1/2002  | Fermaniuk et al.   | 7,013,989 B2 | 3/2006  | Hammond et al.       |
| 6,341,747 B1 | 1/2002  | Schmidt et al.     | 7,013,998 B2 | 3/2006  | Ray et al.           |
| 6,349,766 B1 | 2/2002  | Bussear et al.     | 7,017,664 B2 | 3/2006  | Walker et al.        |
| 6,354,372 B1 | 3/2002  | Carisell et al.    | 7,017,677 B2 | 3/2006  | Keshavan et al.      |
| 6,354,379 B2 | 3/2002  | Miszewski et al.   | 7,021,389 B2 | 4/2006  | Bishop et al.        |
| 6,371,206 B1 | 4/2002  | Mills              | 7,025,146 B2 | 4/2006  | King et al.          |
| 6,372,346 B1 | 4/2002  | Toth               | 7,028,778 B2 | 4/2006  | Krywitsky            |
| 6,382,244 B2 | 5/2002  | Vann               | 7,044,230 B2 | 5/2006  | Starr et al.         |
| 6,390,195 B1 | 5/2002  | Nguyen et al.      | 7,048,812 B2 | 5/2006  | Bettles et al.       |
| 6,390,200 B1 | 5/2002  | Allamon et al.     | 7,049,272 B2 | 5/2006  | Sinclair et al.      |
| 6,394,180 B1 | 5/2002  | Berscheidt et al.  | 7,051,805 B2 | 5/2006  | Doane et al.         |
| 6,394,185 B1 | 5/2002  | Constien           | 7,059,410 B2 | 6/2006  | Bousche et al.       |
| 6,395,402 B1 | 5/2002  | Lambert et al.     | 7,063,748 B2 | 6/2006  | Talton               |
| 6,397,950 B1 | 6/2002  | Streich et al.     | 7,090,027 B1 | 8/2006  | Williams             |
| 6,401,547 B1 | 6/2002  | Hatfield et al.    | 7,093,664 B2 | 8/2006  | Todd et al.          |
| 6,403,210 B1 | 6/2002  | Stuivinga et al.   | 7,096,945 B2 | 8/2006  | Richards et al.      |
| 6,408,946 B1 | 6/2002  | Marshall et al.    | 7,096,946 B2 | 8/2006  | Jasser et al.        |
| 6,419,023 B1 | 7/2002  | George et al.      | 7,097,807 B1 | 8/2006  | Meeks, III et al.    |
| 6,422,314 B1 | 7/2002  | Todd et al.        | 7,097,906 B2 | 8/2006  | Gardner              |
| 6,439,313 B1 | 8/2002  | Thomeer et al.     | 7,108,080 B2 | 9/2006  | Tessari et al.       |
| 6,444,316 B1 | 9/2002  | Reddy et al.       | 7,111,682 B2 | 9/2006  | Blaisdell            |
| 6,446,717 B1 | 9/2002  | White et al.       | 7,128,145 B2 | 10/2006 | Mickey               |
| 6,457,525 B1 | 10/2002 | Scott              | 7,141,207 B2 | 11/2006 | Jandeska, Jr. et al. |
| 6,467,546 B2 | 10/2002 | Allamon et al.     | 7,150,326 B2 | 12/2006 | Bishop et al.        |
| 6,470,965 B1 | 10/2002 | Winzer             | 7,163,066 B2 | 1/2007  | Lehr                 |
| 6,491,097 B1 | 12/2002 | Oneal et al.       | 7,165,622 B2 | 1/2007  | Hirth et al.         |
| 6,491,116 B2 | 12/2002 | Berscheidt et al.  | 7,168,494 B2 | 1/2007  | Starr et al.         |
| 6,513,598 B2 | 2/2003  | Moore et al.       | 7,174,963 B2 | 2/2007  | Bertelsen            |
| 6,513,600 B2 | 2/2003  | Ross               | 7,182,135 B2 | 2/2007  | Szarka               |
| 6,527,051 B1 | 3/2003  | Reddy et al.       | 7,188,559 B1 | 3/2007  | Vecchio              |
| 6,540,033 B1 | 4/2003  | Sullivan et al.    | 7,210,527 B2 | 5/2007  | Walker et al.        |
| 6,543,543 B2 | 4/2003  | Muth               | 7,210,533 B2 | 5/2007  | Starr et al.         |
| 6,554,071 B1 | 4/2003  | Reddy et al.       | 7,217,311 B2 | 5/2007  | Hong et al.          |
| 6,561,275 B2 | 5/2003  | Glass et al.       | 7,234,530 B2 | 6/2007  | Gass                 |
| 6,581,681 B1 | 6/2003  | Zimmerman et al.   | 7,250,188 B2 | 7/2007  | Dodelet et al.       |
| 6,588,507 B2 | 7/2003  | Dusterhoft et al.  | 7,252,162 B2 | 8/2007  | Akinlade et al.      |

(56)

## References Cited

## U.S. PATENT DOCUMENTS

|              |         |                          |              |         |                     |
|--------------|---------|--------------------------|--------------|---------|---------------------|
| 7,267,178 B2 | 9/2007  | Krywitsky                | 7,712,541 B2 | 5/2010  | Loretz et al.       |
| 7,270,186 B2 | 9/2007  | Johnson                  | 7,723,272 B2 | 5/2010  | Crews et al.        |
| 7,287,592 B2 | 10/2007 | Surjaatmadja et al.      | 7,726,406 B2 | 6/2010  | Xu                  |
| 7,311,152 B2 | 12/2007 | Howard et al.            | 7,735,578 B2 | 6/2010  | Loehr et al.        |
| 7,316,274 B2 | 1/2008  | Xu et al.                | 7,743,836 B2 | 6/2010  | Cook et al.         |
| 7,320,365 B2 | 1/2008  | Pia                      | 7,752,971 B2 | 7/2010  | Loehr               |
| 7,322,412 B2 | 1/2008  | Badalamenti et al.       | 7,757,773 B2 | 7/2010  | Rytlewski           |
| 7,322,417 B2 | 1/2008  | Rytlewski et al.         | 7,762,342 B2 | 7/2010  | Richard et al.      |
| 7,325,617 B2 | 2/2008  | Murray                   | 7,770,652 B2 | 8/2010  | Barnett             |
| 7,328,750 B2 | 2/2008  | Swor et al.              | 7,771,289 B2 | 8/2010  | Palumbo et al.      |
| 7,331,388 B2 | 2/2008  | Vilela et al.            | 7,771,547 B2 | 8/2010  | Bieler et al.       |
| 7,337,854 B2 | 3/2008  | Horn et al.              | 7,775,284 B2 | 8/2010  | Richard et al.      |
| 7,346,456 B2 | 3/2008  | Le Bemadjiel             | 7,775,285 B2 | 8/2010  | Surjaatmadja et al. |
| 7,350,582 B2 | 4/2008  | McKeachnie et al.        | 7,775,286 B2 | 8/2010  | Duphorne            |
| 7,353,867 B2 | 4/2008  | Carter et al.            | 7,784,543 B2 | 8/2010  | Johnson             |
| 7,353,879 B2 | 4/2008  | Todd et al.              | 7,793,714 B2 | 9/2010  | Johnson             |
| 7,360,593 B2 | 4/2008  | Constien                 | 7,793,820 B2 | 9/2010  | Hirano et al.       |
| 7,360,597 B2 | 4/2008  | Blaisdell                | 7,794,520 B2 | 9/2010  | Murty et al.        |
| 7,363,970 B2 | 4/2008  | Corre et al.             | 7,798,225 B2 | 9/2010  | Giroux et al.       |
| 7,373,978 B2 | 5/2008  | Barry et al.             | 7,798,226 B2 | 9/2010  | Themig              |
| 7,380,600 B2 | 6/2008  | Willberg et al.          | 7,798,236 B2 | 9/2010  | McKeachnie et al.   |
| 7,384,443 B2 | 6/2008  | Mirchandani              | 7,806,189 B2 | 10/2010 | Frazier             |
| 7,387,158 B2 | 6/2008  | Murray et al.            | 7,806,192 B2 | 10/2010 | Foster et al.       |
| 7,387,165 B2 | 6/2008  | Lopez de Cardenas et al. | 7,810,553 B2 | 10/2010 | Cruickshank et al.  |
| 7,392,841 B2 | 7/2008  | Murray et al.            | 7,810,567 B2 | 10/2010 | Daniels et al.      |
| 7,401,648 B2 | 7/2008  | Richard                  | 7,819,198 B2 | 10/2010 | Birkhead et al.     |
| 7,416,029 B2 | 8/2008  | Telfer et al.            | 7,828,055 B2 | 11/2010 | Willauer et al.     |
| 7,422,058 B2 | 9/2008  | O'Malley                 | 7,833,944 B2 | 11/2010 | Munoz et al.        |
| 7,426,964 B2 | 9/2008  | Lynde et al.             | 7,849,927 B2 | 12/2010 | Herrera             |
| 7,441,596 B2 | 10/2008 | Wood et al.              | 7,851,016 B2 | 12/2010 | Arbab et al.        |
| 7,445,049 B2 | 11/2008 | Howard et al.            | 7,855,168 B2 | 12/2010 | Fuller et al.       |
| 7,451,815 B2 | 11/2008 | Hailey, Jr.              | 7,861,779 B2 | 1/2011  | Vestavik            |
| 7,451,817 B2 | 11/2008 | Reddy et al.             | 7,861,781 B2 | 1/2011  | D'Arcy              |
| 7,461,699 B2 | 12/2008 | Richard et al.           | 7,874,365 B2 | 1/2011  | East, Jr. et al.    |
| 7,464,752 B2 | 12/2008 | Dale et al.              | 7,878,253 B2 | 2/2011  | Stowe et al.        |
| 7,464,764 B2 | 12/2008 | Xu                       | 7,879,162 B2 | 2/2011  | Pandey              |
| 7,472,750 B2 | 1/2009  | Walker et al.            | 7,879,367 B2 | 2/2011  | Heublein et al.     |
| 7,478,676 B2 | 1/2009  | East, Jr. et al.         | 7,896,091 B2 | 3/2011  | Williamson et al.   |
| 7,491,444 B2 | 2/2009  | Smith et al.             | 7,897,063 B1 | 3/2011  | Perry et al.        |
| 7,503,390 B2 | 3/2009  | Gomez                    | 7,900,696 B1 | 3/2011  | Nish et al.         |
| 7,503,392 B2 | 3/2009  | King et al.              | 7,900,703 B2 | 3/2011  | Clark et al.        |
| 7,503,399 B2 | 3/2009  | Badalamenti et al.       | 7,909,096 B2 | 3/2011  | Clarke et al.       |
| 7,509,993 B1 | 3/2009  | Turng et al.             | 7,909,104 B2 | 3/2011  | Bjorgum             |
| 7,510,018 B2 | 3/2009  | Williamson et al.        | 7,909,110 B2 | 3/2011  | Sharma et al.       |
| 7,513,311 B2 | 4/2009  | Gramstad et al.          | 7,909,115 B2 | 3/2011  | Grove et al.        |
| 7,516,791 B2 | 4/2009  | Bryant et al.            | 7,913,765 B2 | 3/2011  | Crow et al.         |
| 7,520,944 B2 | 4/2009  | Johnson                  | 7,918,275 B2 | 4/2011  | Clem                |
| 7,527,103 B2 | 5/2009  | Huang et al.             | 7,931,093 B2 | 4/2011  | Foster et al.       |
| 7,531,020 B2 | 5/2009  | Woodfield et al.         | 7,938,191 B2 | 5/2011  | Vaidya              |
| 7,531,021 B2 | 5/2009  | Woodfield et al.         | 7,946,335 B2 | 5/2011  | Bewlay et al.       |
| 7,537,825 B1 | 5/2009  | Wardle et al.            | 7,946,340 B2 | 5/2011  | Surjattmadja et al. |
| 7,552,777 B2 | 6/2009  | Murray et al.            | 7,958,940 B2 | 6/2011  | Jameson             |
| 7,552,779 B2 | 6/2009  | Murray                   | 7,963,331 B2 | 6/2011  | Surjattmadja et al. |
| 7,559,357 B2 | 7/2009  | Clem                     | 7,963,340 B2 | 6/2011  | Gramstad et al.     |
| 7,575,062 B2 | 8/2009  | East, Jr.                | 7,963,342 B2 | 6/2011  | George              |
| 7,579,087 B2 | 8/2009  | Maloney et al.           | 7,980,300 B2 | 7/2011  | Roberts et al.      |
| 7,591,318 B2 | 9/2009  | Tilghman                 | 7,987,906 B1 | 8/2011  | Troy                |
| 7,600,572 B2 | 10/2009 | Slup et al.              | 7,992,763 B2 | 8/2011  | Vecchio et al.      |
| 7,604,049 B2 | 10/2009 | Vaidya et al.            | 7,999,987 B2 | 8/2011  | Dellinger et al.    |
| 7,604,055 B2 | 10/2009 | Richard et al.           | 8,002,821 B2 | 8/2011  | Stinson             |
| 7,607,476 B2 | 10/2009 | Tom et al.               | 8,020,619 B1 | 9/2011  | Robertson et al.    |
| 7,617,871 B2 | 11/2009 | Surjaatmadja et al.      | 8,020,620 B2 | 9/2011  | Daniels et al.      |
| 7,635,023 B2 | 12/2009 | Goldberg et al.          | 8,025,104 B2 | 9/2011  | Cooke, Jr.          |
| 7,640,988 B2 | 1/2010  | Phi et al.               | 8,028,767 B2 | 10/2011 | Radford et al.      |
| 7,647,964 B2 | 1/2010  | Akbar et al.             | 8,033,331 B2 | 10/2011 | Themig              |
| 7,661,480 B2 | 2/2010  | Al-Anazi                 | 8,034,152 B2 | 10/2011 | Westin et al.       |
| 7,661,481 B2 | 2/2010  | Todd et al.              | 8,039,422 B1 | 10/2011 | Al-Zahrani          |
| 7,665,537 B2 | 2/2010  | Patel et al.             | 8,056,628 B2 | 11/2011 | Whitsitt et al.     |
| 7,686,082 B2 | 3/2010  | Marsh                    | 8,056,638 B2 | 11/2011 | Clayton et al.      |
| 7,690,436 B2 | 4/2010  | Turley et al.            | 8,109,340 B2 | 2/2012  | Doane et al.        |
| 7,699,101 B2 | 4/2010  | Fripp et al.             | 8,114,148 B2 | 2/2012  | Atanasoska et al.   |
| 7,700,038 B2 | 4/2010  | Soran et al.             | 8,119,713 B2 | 2/2012  | Dubois et al.       |
| 7,703,511 B2 | 4/2010  | Buyers et al.            | 8,127,856 B1 | 3/2012  | Nish et al.         |
| 7,708,078 B2 | 5/2010  | Stoesz                   | 8,153,052 B2 | 4/2012  | Jackson et al.      |
| 7,709,421 B2 | 5/2010  | Jones et al.             | 8,163,060 B2 | 4/2012  | Manishi et al.      |
|              |         |                          | 8,167,043 B2 | 5/2012  | Willberg et al.     |
|              |         |                          | 8,211,247 B2 | 7/2012  | Marya et al.        |
|              |         |                          | 8,211,248 B2 | 7/2012  | Marya               |
|              |         |                          | 8,211,331 B2 | 7/2012  | Jorgensen et al.    |

(56)

## References Cited

## U.S. PATENT DOCUMENTS

|              |         |                      |                 |         |                  |
|--------------|---------|----------------------|-----------------|---------|------------------|
| 8,220,554 B2 | 7/2012  | Jordan et al.        | 9,217,319 B2    | 12/2015 | Frazier et al.   |
| 8,226,740 B2 | 7/2012  | Chaumonnot et al.    | 9,227,243 B2    | 1/2016  | Xu et al.        |
| 8,230,731 B2 | 7/2012  | Dyer et al.          | 9,243,475 B2    | 1/2016  | Xu               |
| 8,231,947 B2 | 7/2012  | Vaidya et al.        | 9,260,935 B2    | 2/2016  | Murphree et al.  |
| 8,263,178 B2 | 9/2012  | Boulos et al.        | 9,284,803 B2    | 3/2016  | Stone et al.     |
| 8,267,177 B1 | 9/2012  | Vogel et al.         | 9,309,733 B2    | 4/2016  | Xu et al.        |
| 8,276,670 B2 | 10/2012 | Patel                | 9,309,744 B2    | 4/2016  | Frazier          |
| 8,277,974 B2 | 10/2012 | Kumar et al.         | 9,366,106 B2    | 6/2016  | Xu et al.        |
| 8,297,364 B2 | 10/2012 | Agrawal et al.       | 9,447,482 B2    | 9/2016  | Kim et al.       |
| 8,327,931 B2 | 12/2012 | Agrawal et al.       | 9,458,692 B2    | 10/2016 | Fripp et al.     |
| 8,403,037 B2 | 3/2013  | Agrawal et al.       | 9,500,061 B2    | 11/2016 | Frazier et al.   |
| 8,413,727 B2 | 4/2013  | Holmes               | 9,528,343 B2    | 12/2016 | Jordan et al.    |
| 8,425,651 B2 | 4/2013  | Xu et al.            | 9,587,156 B2    | 3/2017  | Crews            |
| 8,459,347 B2 | 6/2013  | Stout                | 9,605,508 B2    | 3/2017  | Xu               |
| RE44,385 E   | 7/2013  | Johnson              | 9,643,250 B2    | 5/2017  | Mazyar et al.    |
| 8,485,265 B2 | 7/2013  | Marya et al.         | 9,682,425 B2    | 6/2017  | Xu et al.        |
| 8,486,329 B2 | 7/2013  | Shikai et al.        | 9,689,227 B2    | 6/2017  | Fripp et al.     |
| 8,490,674 B2 | 7/2013  | Stevens et al.       | 9,689,231 B2    | 6/2017  | Fripp et al.     |
| 8,490,689 B1 | 7/2013  | McClinton et al.     | 9,789,663 B2    | 10/2017 | Zhang et al.     |
| 8,506,733 B2 | 8/2013  | Enami et al.         | 9,790,763 B2    | 10/2017 | Fripp et al.     |
| 8,528,633 B2 | 9/2013  | Agrawal et al.       | 9,802,250 B2    | 10/2017 | Xu               |
| 8,535,604 B1 | 9/2013  | Baker et al.         | 9,803,439 B2    | 10/2017 | Xu et al.        |
| 8,573,295 B2 | 11/2013 | Johnson et al.       | 9,833,838 B2    | 12/2017 | Mazyar et al.    |
| 8,579,023 B1 | 11/2013 | Nish et al.          | 9,835,016 B2    | 12/2017 | Zhang et al.     |
| 8,613,789 B2 | 12/2013 | Han et al.           | 9,863,201 B2    | 1/2018  | Fripp et al.     |
| 8,631,876 B2 | 1/2014  | Xu et al.            | 9,925,589 B2    | 3/2018  | Xu               |
| 8,663,401 B2 | 3/2014  | Marya et al.         | 9,926,763 B2    | 3/2018  | Mazyar et al.    |
| 8,668,762 B2 | 3/2014  | Kim et al.           | 9,938,451 B2    | 4/2018  | Crews            |
| 8,695,684 B2 | 4/2014  | Chen et al.          | 9,970,249 B2    | 5/2018  | Zhang et al.     |
| 8,695,714 B2 | 4/2014  | Xu                   | 10,016,810 B2   | 7/2018  | Salinas et al.   |
| 8,714,268 B2 | 5/2014  | Agrawal et al.       | 10,059,092 B2   | 8/2018  | Welch et al.     |
| 8,715,339 B2 | 5/2014  | Atanasoska et al.    | 10,059,867 B2   | 8/2018  | Crews            |
| 8,723,564 B2 | 5/2014  | Kim et al.           | 10,081,853 B2   | 9/2018  | Wilks et al.     |
| 8,734,564 B2 | 5/2014  | Kim et al.           | 10,082,008 B2   | 9/2018  | Robey et al.     |
| 8,734,602 B2 | 5/2014  | Li et al.            | 10,092,953 B2   | 10/2018 | Mazyar et al.    |
| 8,746,342 B1 | 6/2014  | Nish et al.          | 10,119,358 B2   | 11/2018 | Walton et al.    |
| 8,770,261 B2 | 7/2014  | Marya                | 10,119,359 B2   | 11/2018 | Frazier          |
| 8,776,884 B2 | 7/2014  | Xu                   | 10,125,565 B2   | 11/2018 | Fripp et al.     |
| 8,789,610 B2 | 7/2014  | Oxford               | 10,167,691 B2   | 1/2019  | Zhang et al.     |
| 8,808,423 B2 | 8/2014  | Kim et al.           | 10,174,578 B2   | 1/2019  | Walton et al.    |
| 8,852,363 B2 | 10/2014 | Numano et al.        | 10,202,820 B2   | 2/2019  | Xu et al.        |
| 8,905,147 B2 | 12/2014 | Fripp et al.         | 10,221,637 B2   | 3/2019  | Xu et al.        |
| 8,950,504 B2 | 2/2015  | Xu et al.            | 10,221,641 B2   | 3/2019  | Zhang et al.     |
| 8,956,660 B2 | 2/2015  | Launag et al.        | 10,221,642 B2   | 3/2019  | Zhang et al.     |
| 8,967,275 B2 | 3/2015  | Crews                | 10,221,643 B2   | 3/2019  | Zhang et al.     |
| 8,978,734 B2 | 3/2015  | Stevens              | 10,227,841 B2   | 3/2019  | Fripp et al.     |
| 8,991,485 B2 | 3/2015  | Chenault et al.      | 10,253,590 B2   | 4/2019  | Xu et al.        |
| 8,998,978 B2 | 4/2015  | Wang                 | 10,266,923 B2   | 4/2019  | Wilks et al.     |
| 9,010,416 B2 | 4/2015  | Xu et al.            | 10,316,601 B2   | 6/2019  | Walton et al.    |
| 9,016,363 B2 | 4/2015  | Xu et al.            | 10,329,643 B2   | 6/2019  | Wilks et al.     |
| 9,016,384 B2 | 4/2015  | Xu                   | 10,335,855 B2   | 7/2019  | Welch et al.     |
| 9,022,107 B2 | 5/2015  | Agrawal et al.       | 10,337,086 B2   | 7/2019  | Wilks et al.     |
| 9,027,655 B2 | 5/2015  | Xu                   | 10,344,568 B2   | 7/2019  | Murphree et al.  |
| 9,033,041 B2 | 5/2015  | Baihly et al.        | 10,364,630 B2   | 7/2019  | Xu et al.        |
| 9,033,060 B2 | 5/2015  | Xu et al.            | 10,364,631 B2   | 7/2019  | Xu et al.        |
| 9,044,397 B2 | 6/2015  | Choi et al.          | 10,364,632 B2   | 7/2019  | Xu et al.        |
| 9,057,117 B2 | 6/2015  | Harrison et al.      | 10,450,840 B2   | 10/2019 | Xu               |
| 9,057,242 B2 | 6/2015  | Mazyar et al.        | 10,472,909 B2   | 11/2019 | Xu et al.        |
| 9,068,428 B2 | 6/2015  | Mazyar et al.        | 10,533,392 B2   | 1/2020  | Walton et al.    |
| 9,010,424 B2 | 7/2015  | Xu                   | 10,544,652 B2   | 1/2020  | Fripp et al.     |
| 9,079,246 B2 | 7/2015  | Xu et al.            | 10,597,965 B2   | 3/2020  | Allen            |
| 9,080,098 B2 | 7/2015  | Xu et al.            | 10,612,659 B2   | 4/2020  | Xu et al.        |
| 9,080,403 B2 | 7/2015  | Xu et al.            | 10,619,438 B2   | 4/2020  | Fripp et al.     |
| 9,080,439 B2 | 7/2015  | O'Malley             | 10,619,445 B2   | 4/2020  | Murphree et al.  |
| 9,089,408 B2 | 7/2015  | Xu                   | 10,626,695 B2   | 4/2020  | Fripp et al.     |
| 9,090,955 B2 | 7/2015  | Xu et al.            | 10,633,947 B2   | 4/2020  | Fripp et al.     |
| 9,090,956 B2 | 7/2015  | Xu                   | 10,655,411 B2   | 5/2020  | Fripp et al.     |
| 9,101,978 B2 | 8/2015  | Xu                   | 10,669,797 B2   | 6/2020  | Johnson et al.   |
| 9,109,429 B2 | 8/2015  | Xu et al.            | 10,724,321 B2   | 7/2020  | Leonard et al.   |
| 9,119,906 B2 | 9/2015  | Tomantschager et al. | 10,737,321 B2   | 8/2020  | Xu               |
| 9,127,515 B2 | 9/2015  | Xu et al.            | 10,781,658 B1   | 9/2020  | Kumar et al.     |
| 9,163,467 B2 | 10/2015 | Gaudette et al.      | 10,807,355 B2   | 10/2020 | Welch et al.     |
| 9,181,088 B2 | 11/2015 | Sibuet et al.        | 2002/0020527 A1 | 2/2002  | Kilaas et al.    |
| 9,187,686 B2 | 11/2015 | Crews                | 2002/0047058 A1 | 4/2002  | Verhoff et al.   |
| 9,211,586 B1 | 12/2015 | Avernia et al.       | 2002/0092654 A1 | 7/2002  | Coronado et al.  |
|              |         |                      | 2002/0104616 A1 | 8/2002  | De et al.        |
|              |         |                      | 2002/0108756 A1 | 8/2002  | Harrall et al.   |
|              |         |                      | 2002/0121081 A1 | 9/2002  | Cesaroni et al.  |
|              |         |                      | 2002/0139541 A1 | 10/2002 | Sheffield et al. |

| (56)                  | References Cited |                      |                 |         |                    |  |  |
|-----------------------|------------------|----------------------|-----------------|---------|--------------------|--|--|
| U.S. PATENT DOCUMENTS |                  |                      |                 |         |                    |  |  |
| 2002/0197181 A1       | 12/2002          | Osawa et al.         | 2007/0181224 A1 | 8/2007  | Marya et al.       |  |  |
| 2003/0019639 A1       | 1/2003           | Mackay               | 2007/0187095 A1 | 8/2007  | Walker et al.      |  |  |
| 2003/0060374 A1       | 3/2003           | Cooke, Jr.           | 2007/0207182 A1 | 9/2007  | Weber et al.       |  |  |
| 2003/0104147 A1       | 6/2003           | Bretschneider et al. | 2007/0221373 A1 | 9/2007  | Murray             |  |  |
| 2003/0111728 A1       | 6/2003           | Thai et al.          | 2007/0227745 A1 | 10/2007 | Roberts et al.     |  |  |
| 2003/0127013 A1       | 7/2003           | Zavitsanos et al.    | 2007/0259994 A1 | 11/2007 | Tour et al.        |  |  |
| 2003/0141060 A1       | 7/2003           | Hailey, Jr. et al.   | 2007/0270942 A1 | 11/2007 | Thomas             |  |  |
| 2003/0150614 A1       | 8/2003           | Brown et al.         | 2007/0284112 A1 | 12/2007 | Magne et al.       |  |  |
| 2003/0155114 A1       | 8/2003           | Pedersen et al.      | 2007/0299510 A1 | 12/2007 | Venkatraman et al. |  |  |
| 2003/0173005 A1       | 9/2003           | Higashi              | 2008/0011473 A1 | 1/2008  | Wood et al.        |  |  |
| 2004/0005483 A1       | 1/2004           | Lin                  | 2008/0020923 A1 | 1/2008  | Debe et al.        |  |  |
| 2004/0055758 A1       | 3/2004           | Brezinski et al.     | 2008/0041500 A1 | 2/2008  | Bronfin            |  |  |
| 2004/0069502 A1       | 4/2004           | Luke                 | 2008/0047707 A1 | 2/2008  | Boney et al.       |  |  |
| 2004/0089449 A1       | 5/2004           | Walton et al.        | 2008/0060810 A9 | 3/2008  | Nguyen et al.      |  |  |
| 2004/0094297 A1       | 5/2004           | Malone et al.        | 2008/0081866 A1 | 4/2008  | Gong et al.        |  |  |
| 2004/0154806 A1       | 8/2004           | Bode et al.          | 2008/0093073 A1 | 4/2008  | Bustos et al.      |  |  |
| 2004/0159446 A1       | 8/2004           | Haugen et al.        | 2008/0121436 A1 | 5/2008  | Slay et al.        |  |  |
| 2004/0216868 A1       | 11/2004          | Owens, Sr.           | 2008/0127475 A1 | 6/2008  | Griffo             |  |  |
| 2004/0231845 A1       | 11/2004          | Cooke, Jr.           | 2008/0149325 A1 | 6/2008  | Crawford           |  |  |
| 2004/0244968 A1       | 12/2004          | Cook et al.          | 2008/0149345 A1 | 6/2008  | Marya et al.       |  |  |
| 2004/0256109 A1       | 12/2004          | Johnson              | 2008/0149351 A1 | 6/2008  | Marya et al.       |  |  |
| 2004/0261993 A1       | 12/2004          | Nguyen               | 2008/0169130 A1 | 7/2008  | Norman et al.      |  |  |
| 2004/0261994 A1       | 12/2004          | Nguyen et al.        | 2008/0175744 A1 | 7/2008  | Motegi             |  |  |
| 2005/0064247 A1       | 3/2005           | Sane et al.          | 2008/0179104 A1 | 7/2008  | Zhang et al.       |  |  |
| 2005/0074612 A1       | 4/2005           | Eklund et al.        | 2008/0196801 A1 | 8/2008  | Zhao et al.        |  |  |
| 2005/0098313 A1       | 5/2005           | Atkins et al.        | 2008/0202764 A1 | 8/2008  | Clayton et al.     |  |  |
| 2005/0102255 A1       | 5/2005           | Bultman              | 2008/0202814 A1 | 8/2008  | Lyons et al.       |  |  |
| 2005/0106316 A1       | 5/2005           | Rigney et al.        | 2008/0210473 A1 | 9/2008  | Zhang et al.       |  |  |
| 2005/0161212 A1       | 7/2005           | Leismer et al.       | 2008/0216383 A1 | 9/2008  | Pierick et al.     |  |  |
| 2005/0165149 A1       | 7/2005           | Chanak et al.        | 2008/0220991 A1 | 9/2008  | Slay et al.        |  |  |
| 2005/0194141 A1       | 9/2005           | Sinclair et al.      | 2008/0223587 A1 | 9/2008  | Cherewyk           |  |  |
| 2005/0235757 A1       | 10/2005          | De Jonge et al.      | 2008/0236829 A1 | 10/2008 | Lynde              |  |  |
| 2005/0241824 A1       | 11/2005          | Burris, II et al.    | 2008/0236842 A1 | 10/2008 | Bhavsar et al.     |  |  |
| 2005/0241825 A1       | 11/2005          | Burris, II et al.    | 2008/0248205 A1 | 10/2008 | Blanchet et al.    |  |  |
| 2005/0268746 A1       | 12/2005          | Abkowitz et al.      | 2008/0248413 A1 | 10/2008 | Ishii et al.       |  |  |
| 2005/0269097 A1       | 12/2005          | Towler               | 2008/0264205 A1 | 10/2008 | Zeng et al.        |  |  |
| 2005/0275143 A1       | 12/2005          | Toth                 | 2008/0264594 A1 | 10/2008 | Lohmueller et al.  |  |  |
| 2005/0279427 A1       | 12/2005          | Park et al.          | 2008/0277980 A1 | 11/2008 | Koda et al.        |  |  |
| 2005/0279501 A1       | 12/2005          | Surjaatmadja et al.  | 2008/0282924 A1 | 11/2008 | Saenger et al.     |  |  |
| 2006/0012087 A1       | 1/2006           | Matsuda et al.       | 2008/0296024 A1 | 12/2008 | Huang et al.       |  |  |
| 2006/0013350 A1       | 1/2006           | Akers                | 2008/0302538 A1 | 12/2008 | Hofman             |  |  |
| 2006/0057479 A1       | 3/2006           | Niimi et al.         | 2008/0314581 A1 | 12/2008 | Brown              |  |  |
| 2006/0102871 A1       | 5/2006           | Wang et al.          | 2008/0314588 A1 | 12/2008 | Langlais et al.    |  |  |
| 2006/0108114 A1       | 5/2006           | Johnson              | 2009/0038858 A1 | 2/2009  | Griffo et al.      |  |  |
| 2006/0110615 A1       | 5/2006           | Karim et al.         | 2009/0044946 A1 | 2/2009  | Shasteen et al.    |  |  |
| 2006/0113077 A1       | 6/2006           | Willberg et al.      | 2009/0044955 A1 | 2/2009  | King et al.        |  |  |
| 2006/0116696 A1       | 6/2006           | Odermatt et al.      | 2009/0050334 A1 | 2/2009  | Marya et al.       |  |  |
| 2006/0131031 A1       | 6/2006           | McKeachnie           | 2009/0056934 A1 | 3/2009  | Xu                 |  |  |
| 2006/0131081 A1       | 6/2006           | Mirchandani et al.   | 2009/0065216 A1 | 3/2009  | Frazier            |  |  |
| 2006/0144515 A1       | 7/2006           | Tada et al.          | 2009/0068051 A1 | 3/2009  | Gross              |  |  |
| 2006/0150770 A1       | 7/2006           | Freim, III et al.    | 2009/0074603 A1 | 3/2009  | Chan et al.        |  |  |
| 2006/0153728 A1       | 7/2006           | Schoenung et al.     | 2009/0084600 A1 | 4/2009  | Severance          |  |  |
| 2006/0169453 A1       | 8/2006           | Savery et al.        | 2009/0090440 A1 | 4/2009  | Kellett            |  |  |
| 2006/0175059 A1       | 8/2006           | Sinclair et al.      | 2009/0107684 A1 | 4/2009  | Cooke, Jr.         |  |  |
| 2006/0186602 A1       | 8/2006           | Martin et al.        | 2009/0114381 A1 | 5/2009  | Stroobants         |  |  |
| 2006/0207387 A1       | 9/2006           | Soran et al.         | 2009/0116992 A1 | 5/2009  | Lee                |  |  |
| 2006/0269437 A1       | 11/2006          | Pandey               | 2009/0126436 A1 | 5/2009  | Fly et al.         |  |  |
| 2006/0278405 A1       | 12/2006          | Turley               | 2009/0151949 A1 | 6/2009  | Marya et al.       |  |  |
| 2006/0283592 A1       | 12/2006          | Sierra et al.        | 2009/0152009 A1 | 6/2009  | Slay et al.        |  |  |
| 2007/0017675 A1       | 1/2007           | Hammami et al.       | 2009/0155616 A1 | 6/2009  | Thamida            |  |  |
| 2007/0134496 A1       | 1/2007           | Katagiri et al.      | 2009/0159289 A1 | 6/2009  | Avant et al.       |  |  |
| 2007/0039161 A1       | 2/2007           | Garcia               | 2009/0194745 A1 | 8/2009  | Tanaka             |  |  |
| 2007/0044958 A1       | 3/2007           | Rytlewski et al.     | 2009/0205841 A1 | 8/2009  | Kluge et al.       |  |  |
| 2007/0044966 A1       | 3/2007           | Davies et al.        | 2009/0211770 A1 | 8/2009  | Nutley et al.      |  |  |
| 2007/0051521 A1       | 3/2007           | Fike et al.          | 2009/0226340 A1 | 9/2009  | Marya              |  |  |
| 2007/0053785 A1       | 3/2007           | Hetz et al.          | 2009/0226704 A1 | 9/2009  | Kauppinen et al.   |  |  |
| 2007/0054101 A1       | 3/2007           | Sigalas et al.       | 2009/0242202 A1 | 10/2009 | Rispler et al.     |  |  |
| 2007/0057415 A1       | 3/2007           | Katagiri et al.      | 2009/0242208 A1 | 10/2009 | Bolding            |  |  |
| 2007/0062644 A1       | 3/2007           | Nakamura et al.      | 2009/0255667 A1 | 10/2009 | Clem et al.        |  |  |
| 2007/0102199 A1       | 5/2007           | Smith et al.         | 2009/0255684 A1 | 10/2009 | Bolding            |  |  |
| 2007/0107899 A1       | 5/2007           | Werner et al.        | 2009/0255686 A1 | 10/2009 | Richard et al.     |  |  |
| 2007/0108060 A1       | 5/2007           | Park                 | 2009/0260817 A1 | 10/2009 | Gambier et al.     |  |  |
| 2007/0131912 A1       | 6/2007           | Simone et al.        | 2009/0266548 A1 | 10/2009 | Olsen et al.       |  |  |
| 2007/0151009 A1       | 7/2007           | Conrad, III et al.   | 2009/0272544 A1 | 11/2009 | Giroux et al.      |  |  |
| 2007/0151769 A1       | 7/2007           | Slutz et al.         | 2009/0283270 A1 | 11/2009 | Langeslag          |  |  |
|                       |                  |                      | 2009/0293672 A1 | 12/2009 | Mirchandani et al. |  |  |
|                       |                  |                      | 2009/0301730 A1 | 12/2009 | Gweily             |  |  |
|                       |                  |                      | 2009/0308588 A1 | 12/2009 | Howell et al.      |  |  |
|                       |                  |                      | 2009/0317556 A1 | 12/2009 | Macary             |  |  |

| (56)                  | References Cited |                   |                 |         |                  |  |
|-----------------------|------------------|-------------------|-----------------|---------|------------------|--|
| U.S. PATENT DOCUMENTS |                  |                   |                 |         |                  |  |
| 2009/0317622 A1       | 12/2009          | Huang et al.      | 2012/0177905 A1 | 7/2012  | Seals et al.     |  |
| 2010/0003536 A1       | 1/2010           | Smith et al.      | 2012/0190593 A1 | 7/2012  | Soane et al.     |  |
| 2010/0012385 A1       | 1/2010           | Drivdahl et al.   | 2012/0205120 A1 | 8/2012  | Howell           |  |
| 2010/0015002 A1       | 1/2010           | Barrera et al.    | 2012/0205872 A1 | 8/2012  | Reinhardt et al. |  |
| 2010/0015469 A1       | 1/2010           | Romanowski        | 2012/0211239 A1 | 8/2012  | Kritzler et al.  |  |
| 2010/0025255 A1       | 2/2010           | Si et al.         | 2012/0234546 A1 | 9/2012  | Xu               |  |
| 2010/0038076 A1       | 2/2010           | Spray et al.      | 2012/0234547 A1 | 9/2012  | O'Malley et al.  |  |
| 2010/0038595 A1       | 2/2010           | Imholt et al.     | 2012/0247765 A1 | 10/2012 | Agrawal et al.   |  |
| 2010/0040180 A1       | 2/2010           | Kim et al.        | 2012/0267101 A1 | 10/2012 | Cooke, Jr.       |  |
| 2010/0044041 A1       | 2/2010           | Smith et al.      | 2012/0269673 A1 | 10/2012 | Koo et al.       |  |
| 2010/0051278 A1       | 3/2010           | Mytopher et al.   | 2012/0273229 A1 | 11/2012 | Xu et al.        |  |
| 2010/0055492 A1       | 3/2010           | Baroum et al.     | 2012/0318513 A1 | 12/2012 | Mazyar et al.    |  |
| 2010/0089583 A1       | 4/2010           | Xu et al.         | 2013/0000985 A1 | 1/2013  | Agrawal et al.   |  |
| 2010/0116495 A1       | 5/2010           | Spray             | 2013/0008671 A1 | 1/2013  | Booth            |  |
| 2010/0119405 A1       | 5/2010           | Okamoto et al.    | 2013/0017610 A1 | 1/2013  | Roberts et al.   |  |
| 2010/0139930 A1       | 6/2010           | Patel et al.      | 2013/0022816 A1 | 1/2013  | Smith et al.     |  |
| 2010/0161031 A1       | 6/2010           | Papirov et al.    | 2013/0029886 A1 | 1/2013  | Mazyar et al.    |  |
| 2010/0200230 A1       | 8/2010           | East, Jr. et al.  | 2013/0032357 A1 | 2/2013  | Mazyar et al.    |  |
| 2010/0236793 A1       | 9/2010           | Bjorgum           | 2013/0043041 A1 | 2/2013  | McCoy et al.     |  |
| 2010/0236794 A1       | 9/2010           | Duan et al.       | 2013/0047785 A1 | 2/2013  | Xu               |  |
| 2010/0243254 A1       | 9/2010           | Murphy et al.     | 2013/0052472 A1 | 2/2013  | Xu               |  |
| 2010/0252273 A1       | 10/2010          | Duphorne          | 2013/0056215 A1 | 3/2013  | Crews            |  |
| 2010/0252280 A1       | 10/2010          | Swor et al.       | 2013/0068411 A1 | 3/2013  | Forde et al.     |  |
| 2010/0270031 A1       | 10/2010          | Patel             | 2013/0068461 A1 | 3/2013  | Maerz et al.     |  |
| 2010/0276136 A1       | 11/2010          | Evans et al.      | 2013/0084643 A1 | 4/2013  | Commarieu et al. |  |
| 2010/0276159 A1       | 11/2010          | Mailand et al.    | 2013/0105159 A1 | 5/2013  | Alvarez et al.   |  |
| 2010/0282338 A1       | 11/2010          | Gerrard et al.    | 2013/0112429 A1 | 5/2013  | Crews            |  |
| 2010/0282469 A1       | 11/2010          | Richard et al.    | 2013/0126190 A1 | 5/2013  | Mazyar et al.    |  |
| 2010/0297432 A1       | 11/2010          | Sherman et al.    | 2013/0133897 A1 | 5/2013  | Bailhly et al.   |  |
| 2010/0304178 A1       | 12/2010          | Dirscherl         | 2013/0144290 A1 | 6/2013  | Schiffl et al.   |  |
| 2010/0304182 A1       | 12/2010          | Facchini et al.   | 2013/0146144 A1 | 6/2013  | Joseph et al.    |  |
| 2010/0314105 A1       | 12/2010          | Rose              | 2013/0160992 A1 | 6/2013  | Agrawal et al.   |  |
| 2010/0314127 A1       | 12/2010          | Swor et al.       | 2013/0167502 A1 | 7/2013  | Wilson et al.    |  |
| 2010/0319427 A1       | 12/2010          | Lohbeck et al.    | 2013/0168257 A1 | 7/2013  | Mazyar et al.    |  |
| 2010/0326650 A1       | 12/2010          | Tran et al.       | 2013/0186626 A1 | 7/2013  | Aitken et al.    |  |
| 2011/0005773 A1       | 1/2011           | Dusterhoft et al. | 2013/0199800 A1 | 8/2013  | Kellner et al.   |  |
| 2011/0036592 A1       | 2/2011           | Fay               | 2013/0209308 A1 | 8/2013  | Mazyar et al.    |  |
| 2011/0048743 A1       | 3/2011           | Stafford et al.   | 2013/0204096 A1 | 8/2013  | Noue et al.      |  |
| 2011/0052805 A1       | 3/2011           | Bordere et al.    | 2013/0240200 A1 | 9/2013  | Frazier          |  |
| 2011/0067872 A1       | 3/2011           | Agrawal           | 2013/0240203 A1 | 9/2013  | Frazier          |  |
| 2011/0067889 A1       | 3/2011           | Marya et al.      | 2013/0261735 A1 | 10/2013 | Pacetti et al.   |  |
| 2011/0091660 A1       | 4/2011           | Dirscherl         | 2013/0277044 A1 | 10/2013 | King et al.      |  |
| 2011/0094406 A1       | 4/2011           | Marya et al.      | 2013/0310961 A1 | 11/2013 | Velez            |  |
| 2011/0135530 A1       | 6/2011           | Xu et al.         | 2013/0048289 A1 | 12/2013 | Mazyar           |  |
| 2011/0135805 A1       | 6/2011           | Doucet et al.     | 2013/0319668 A1 | 12/2013 | Tschetter et al. |  |
| 2011/0139465 A1       | 6/2011           | Tibbles et al.    | 2013/0327540 A1 | 12/2013 | Hamid et al.     |  |
| 2011/0147014 A1       | 6/2011           | Chen et al.       | 2014/0018489 A1 | 1/2014  | Johnson          |  |
| 2011/0186306 A1       | 8/2011           | Marya et al.      | 2014/0020712 A1 | 1/2014  | Benson           |  |
| 2011/0192613 A1       | 8/2011           | Garcia et al.     | 2014/0027128 A1 | 1/2014  | Johnson          |  |
| 2011/0214881 A1       | 9/2011           | Newton et al.     | 2014/0060834 A1 | 3/2014  | Quintero         |  |
| 2011/0221137 A1       | 9/2011           | Obi et al.        | 2014/0093417 A1 | 4/2014  | Liu              |  |
| 2011/0236249 A1       | 9/2011           | Kim et al.        | 2014/0110112 A1 | 4/2014  | Jordan, Jr.      |  |
| 2011/0247833 A1       | 10/2011          | Todd et al.       | 2014/0116711 A1 | 5/2014  | Tang             |  |
| 2011/0253387 A1       | 10/2011          | Ervin             | 2014/0124216 A1 | 5/2014  | Fripp et al.     |  |
| 2011/0259610 A1       | 10/2011          | Shhkurti et al.   | 2014/0154341 A1 | 6/2014  | Manuel et al.    |  |
| 2011/0277987 A1       | 11/2011          | Frazier           | 2014/0186207 A1 | 7/2014  | Bae et al.       |  |
| 2011/0277989 A1       | 11/2011          | Frazier           | 2014/0190705 A1 | 7/2014  | Fripp            |  |
| 2011/0277996 A1       | 11/2011          | Cullick et al.    | 2014/0196889 A1 | 7/2014  | Jordan et al.    |  |
| 2011/0284232 A1       | 11/2011          | Huang             | 2014/0202284 A1 | 7/2014  | Kim              |  |
| 2011/0284240 A1       | 11/2011          | Chen et al.       | 2014/0202708 A1 | 7/2014  | Jacob et al.     |  |
| 2011/0284243 A1       | 11/2011          | Frazier           | 2014/0219861 A1 | 8/2014  | Han              |  |
| 2011/0300403 A1       | 12/2011          | Vecchio et al.    | 2014/0224477 A1 | 8/2014  | Wiese et al.     |  |
| 2011/0314881 A1       | 12/2011          | Hatcher et al.    | 2014/0236284 A1 | 8/2014  | Stinson          |  |
| 2012/0046732 A1       | 2/2012           | Sillekens et al.  | 2014/0271333 A1 | 9/2014  | Kim et al.       |  |
| 2012/0067426 A1       | 3/2012           | Soni et al.       | 2014/0286810 A1 | 9/2014  | Marya            |  |
| 2012/0080189 A1       | 4/2012           | Marya et al.      | 2014/0305627 A1 | 10/2014 | Manke            |  |
| 2012/0090839 A1       | 4/2012           | Rudic             | 2014/0311731 A1 | 10/2014 | Smith            |  |
| 2012/0097384 A1       | 4/2012           | Valencia et al.   | 2014/0311752 A1 | 10/2014 | Streich et al.   |  |
| 2012/0103135 A1       | 5/2012           | Xu et al.         | 2014/0360728 A1 | 12/2014 | Tashiro et al.   |  |
| 2012/0125642 A1       | 5/2012           | Chenault          | 2014/0374086 A1 | 12/2014 | Agrawal et al.   |  |
| 2012/0130470 A1       | 5/2012           | Agnew et al.      | 2015/0060085 A1 | 3/2015  | Xu               |  |
| 2012/0145378 A1       | 6/2012           | Frazier           | 2015/0065401 A1 | 3/2015  | Xu et al.        |  |
| 2012/0145389 A1       | 6/2012           | Fitzpatrick, Jr.  | 2015/0102179 A1 | 4/2015  | McHenry et al.   |  |
| 2012/0156087 A1       | 6/2012           | Kawabata          | 2015/0184485 A1 | 7/2015  | Xu et al.        |  |
| 2012/0168152 A1       | 7/2012           | Casciaro          | 2015/0240337 A1 | 8/2015  | Sherman et al.   |  |
|                       |                  |                   | 2015/0247376 A1 | 9/2015  | Tolman et al.    |  |
|                       |                  |                   | 2015/0299838 A1 | 10/2015 | Doud             |  |
|                       |                  |                   | 2015/0354311 A1 | 12/2015 | Okura et al.     |  |
|                       |                  |                   | 2016/0024619 A1 | 1/2016  | Wilks            |  |

| (56)                     | References Cited |         |                      |    |             |         |
|--------------------------|------------------|---------|----------------------|----|-------------|---------|
| U.S. PATENT DOCUMENTS    |                  |         |                      |    |             |         |
| 2016/0128849             | A1               | 5/2016  | Yan et al.           | JP | 2004154837  | 6/2004  |
| 2016/0201425             | A1               | 7/2016  | Walton               | JP | 2004225084  | 8/2004  |
| 2016/0201427             | A1               | 7/2016  | Fripp                | JP | 2004225765  | 8/2004  |
| 2016/0201435             | A1               | 7/2016  | Fripp et al.         | JP | 2005076052  | 3/2005  |
| 2016/0209391             | A1               | 7/2016  | Zhang et al.         | JP | 2008266734  | 11/2008 |
| 2016/0230494             | A1               | 8/2016  | Fripp et al.         | JP | 2008280565  | 11/2008 |
| 2016/0251934             | A1               | 9/2016  | Walton               | JP | 2009144207  | 7/2009  |
| 2016/0258242             | A1               | 9/2016  | Hayter et al.        | JP | 2010502840  | 1/2010  |
| 2016/0265091             | A1               | 9/2016  | Walton et al.        | JP | 2012197491  | 10/2012 |
| 2016/0272882             | A1               | 9/2016  | Stray et al.         | KR | 20130023707 | 3/2013  |
| 2016/0279709             | A1               | 9/2016  | Xu et al.            | NO | 2013109287  | 7/2013  |
| 2017/0050159             | A1               | 2/2017  | Xu et al.            | RU | 2373375     | 7/2006  |
| 2017/0266923             | A1               | 9/2017  | Guest et al.         | WO | 9111587     | 8/1881  |
| 2017/0356266             | A1               | 12/2017 | Arackakudiyil et al. | WO | 1990002655  | 3/1990  |
| 2018/0010217             | A1               | 1/2018  | Wilks et al.         | WO | 9200961     | 1/1992  |
| 2018/0023359             | A1               | 1/2018  | Xu                   | WO | 1992013978  | 8/1992  |
| 2018/0178289             | A1               | 6/2018  | Xu et al.            | WO | 9857347     | 12/1998 |
| 2018/0187510             | A1               | 7/2018  | Xu et al.            | WO | 9909227     | 2/1999  |
| 2018/0216431             | A1               | 8/2018  | Walton et al.        | WO | 1999027146  | 6/1999  |
| 2018/0274317             | A1               | 9/2018  | Hall                 | WO | 9947726     | 9/1999  |
| 2019/0054523             | A1               | 2/2019  | Wolf et al.          | WO | 2001001087  | 1/2001  |
| 2019/0093450             | A1               | 3/2019  | Walton et al.        | WO | 2004001087  | 12/2003 |
| 2019/0203563             | A1               | 7/2019  | Gano et al.          | WO | 20040473889 | 9/2004  |
| 2019/0249510             | A1               | 8/2019  | Deng et al.          | WO | 2005065281  | 7/2005  |
|                          |                  |         |                      | WO | 2007044635  | 4/2007  |
|                          |                  |         |                      | WO | 2007095376  | 8/2007  |
|                          |                  |         |                      | WO | 2008017156  | 2/2008  |
|                          |                  |         |                      | WO | 2008034042  | 3/2008  |
|                          |                  |         |                      | WO | 2008057045  | 5/2008  |
|                          |                  |         |                      | WO | 2008079485  | 7/2008  |
| FOREIGN PATENT DOCUMENTS |                  |         |                      |    |             |         |
| CA                       | 2886988          | 10/2015 |                      | WO | 2008079777  | 7/2008  |
| CN                       | 1076968          | 10/1993 |                      | WO | 2008142129  | 11/2008 |
| CN                       | 1079234          | 12/1993 |                      | WO | 2009055354  | 4/2009  |
| CN                       | 1255879          | 6/2000  |                      | WO | 2009079745  | 7/2009  |
| CN                       | 1668545          | 9/2005  |                      | WO | 2009093420  | 7/2009  |
| CN                       | 1882759          | 12/2006 |                      | WO | 2010012184  | 2/2010  |
| CN                       | 101050417        | 10/2007 |                      | WO | 2010038016  | 4/2010  |
| CN                       | 101351523        | 1/2009  |                      | WO | 2010083826  | 7/2010  |
| CN                       | 101381829        | 3/2009  |                      | WO | 2010110505  | 9/2010  |
| CN                       | 101392345        | 3/2009  |                      | WO | 2011071902  | 6/2011  |
| CN                       | 101454074        | 6/2009  |                      | WO | 2011071907  | 6/2011  |
| CN                       | 101457321        | 6/2009  |                      | WO | 2011071910  | 6/2011  |
| CN                       | 101605963        | 12/2009 |                      | WO | 2011130063  | 10/2011 |
| CN                       | 101720378        | 6/2010  |                      | WO | 2012015567  | 2/2012  |
| CN                       | 102517489        | 6/2012  |                      | WO | 2012071449  | 5/2012  |
| CN                       | 102796928        | 11/2012 |                      | WO | 2012091984  | 7/2012  |
| CN                       | 103343271        | 10/2013 |                      | WO | 2012149007  | 11/2012 |
| CN                       | 103602865        | 2/2014  |                      | WO | 2012164236  | 12/2012 |
| CN                       | 103898384        | 7/2014  |                      | WO | 2012174101  | 12/2012 |
| CN                       | 104004950        | 8/2014  |                      | WO | 2012175665  | 12/2012 |
| CN                       | 104152775        | 11/2014 |                      | WO | 2013019410  | 2/2013  |
| CN                       | 104480354        | 4/2015  |                      | WO | 2013019421  | 2/2013  |
| CN                       | 201532089        | 4/2015  |                      | WO | 2013053057  | 4/2013  |
| CN                       | 104651692        | 5/2015  |                      | WO | 2013078031  | 5/2013  |
| CN                       | 10577976         | 7/2016  |                      | WO | 2013122712  | 8/2013  |
| CN                       | 106086559        | 11/2016 |                      | WO | 2013154634  | 10/2013 |
| EA                       | 200600343        | 6/2006  |                      | WO | 2014100141  | 6/2014  |
| EA                       | 200870227        | 2/2009  |                      | WO | 2014113058  | 7/2014  |
| EP                       | 0033625          | 8/1981  |                      | WO | 2014121384  | 8/2014  |
| EP                       | 0400574          | 5/1990  |                      | WO | 2014210283  | 12/2014 |
| EP                       | 0470599          | 2/1998  |                      | WO | 2015127177  | 8/2015  |
| EP                       | 1006258          | 1/2000  |                      | WO | 2015142862  | 9/2015  |
| EP                       | 1174385          | 1/2002  |                      | WO | 2015161171  | 10/2015 |
| EP                       | 1412175          | 4/2004  |                      | WO | 2015171126  | 11/2015 |
| EP                       | 1493517          | 1/2005  |                      | WO | 2015171585  | 11/2015 |
| EP                       | 1798301          | 6/2007  |                      | WO | 2016024974  | 2/2016  |
| EP                       | 1857570          | 11/2007 |                      | WO | 2016032490  | 3/2016  |
| EP                       | 2088217          | 8/2009  |                      | WO | 2016032493  | 3/2016  |
| GB                       | 912956           | 12/1962 |                      | WO | 2016032619  | 3/2016  |
| GB                       | 1046330          | 10/1966 |                      | WO | 2016032620  | 3/2016  |
| GB                       | 1280833          | 7/1972  |                      | WO | 2016032621  | 3/2016  |
| GB                       | 1357065          | 6/1974  |                      | WO | 2016032758  | 3/2016  |
| GB                       | 2095288          | 9/1982  |                      | WO | 2016032761  | 3/2016  |
| GB                       | 2529062          | 2/2016  |                      | WO | 2016036371  | 3/2016  |
| JP                       | H10147830        | 6/1998  |                      | WO | 2016085798  | 6/2016  |
| JP                       | 2000073152       | 3/2000  |                      |    |             |         |
| JP                       | 2000185725       | 7/2000  |                      |    |             |         |
| JP                       | 2002053902       | 2/2002  |                      |    |             |         |

(56)

## References Cited

## FOREIGN PATENT DOCUMENTS

- WO 2016165041 10/2016  
 WO 2020018110 1/2020  
 WO 2020109770 6/2020

## OTHER PUBLICATIONS

- Hillis et al., "High Purity Magnesium AM60 Alloy: The Critical Contaminant Limits and the Salt Water Corrosion Performance", SAE Technical Paper Series (1986).
- Pawar, S.G., "Influence of Microstructure on the Corrosion Behaviour of Magnesium Alloys", PhD Dissertation, University of Manchester (2011).
- Czerwinski, "Magnesium Injection Molding"; Technology & Engineering; Springer Science + Media, LLC, pp. 107-108, (Dec. 2007).
- Metals Handbook, Desk Edition, edited by J.R. David, published by ASM International, pp. 559-574 (1998).
- Hassan et al., "Development of high strength magnesium based composites using elemental nickel particulates as reinforcement", Journal of Materials Science, vol. 37, pp. 2467-2474 (2002).
- Machine Translation of CN103898384 (originally submitted in Information Disclosure Statement filed Sep. 24, 2020).
- Machine Translation of KR 20130023707 (originally cited in Information Disclosure Statement filed Sep. 24, 2020).
- Machine Translation of CN103602865 (originally cited in Information Disclosure Statement filed Sep. 24, 2020).
- Machine Translation of CN101381829 (originally cited in Information Disclosure Statement filed Sep. 11, 2020).
- Machine Translation of CN102518489 (originally cited in Information Disclosure Statement filed Sep. 11, 2020).
- Machine Translation of CN 103343271 (originally cited in Information Disclosure Statement filed Sep. 11, 2020).
- Machine Translation of CN102796928 (originally cited in Information Disclosure Statement filed Sep. 11, 2020).
- Machine Translation of JP2008266734 (originally cited in Information Disclosure Statement filed Sep. 11, 2020).
- Machine Translation of JP2012197491 (originally cited in Information Disclosure Statement filed Sep. 11, 2020).
- Machine Translation of JP2013019030 (originally cited in Information Disclosure Statement filed Sep. 11, 2020).
- Machine Translation of JP2014043601 (originally cited in Information Disclosure Statement filed Sep. 11, 2020).
- Machine Translation of CN104004950 (See Foreign Patent Document # 2).
- Machine Translation of CN104651691 (See Foreign Patent Document # 3).
- United States District Court / Western District of Oklahoma, Case No. 5:21-cv-1115, *Magnesium Machine LLC v. Terves LLC*, Docket Report (Jan. 24, 2023).
- United States District Court/ Northern District of Ohio, Case No. 1:19-cv-1611, *Terves LLC v. Yueyang Aerospace New Materials Co. Ltd.*, Partial Docket Report (Jan. 24, 2023).
- U.S. Court of Appeals / Federal District, *Terves LLC v. Yueyang Aerospace New Materials Co. Ltd.*, Docket Report (Jan. 24, 2023).
- United States District Court / West District of Oklahoma, Case No. 5:21-cv-1115, *Magnesium Machine, LLC v. Terves LLC*, "Complaint for Declaration Judgment of Non-Infringement, Invalidity, and Unenforceability of Patents, Tortious Interference Contract and Prospective Economic Advantage and Unfair Competition" (Nov. 23, 2021).
- United States District Court / Northern District of Ohio, Eastern Division, Case No. 1:19-cv-1611, *Terves LLC v. Yueyang Aerospace New Materials Co. Ltd.*, "Memorandum in Support of Defendants' Motion for Summary Judgment" (Nov. 18, 2021).
- Patent Trial and Appeal Board / Federal District, *Chongqing Yanmei Technology Co., LTD v. Terves LLC*; Declaration Under 37 CFR 1.68 of Dr. Juan C. Nava, Ph.D. (filed Jan. 24, 2023).
- Curriculum Vitae of Dr. Juan C. Nava, Ph.D.
- Patent Trial and Appeal Board / Federal District, *Chongqing Yanmei Technology Co., LTD v. Terves LLC*; "Petition for Inter Partes Review of U.S. Pat. No. 10,689,740" (filed Jan. 24, 2023).
- Sigworth et al. "Grain Refinement of Aluminum Castings Alloys" American Foundry Society; Paper 07-67; pp. 5-7 (2007).
- Momentive, "Titanium Diborid Powder" condensed product brochure; retrieved from <https://www.momentive.com/WorkArea/DownloadAsset.aspx?id=27489>; p. 1 (2012).
- Durbin, "Modeling Dissolution in Aluminum Alloys" Dissertation for Georgia Institute of Technology; retrieved from [https://smartech.gatech.edu/bitstream/handle/1853/6873/durbin\\_tracie\\_L\\_200505\\_phd.pdf](https://smartech.gatech.edu/bitstream/handle/1853/6873/durbin_tracie_L_200505_phd.pdf) (2005).
- Pegeut et al., "Influence of cold working on the pitting corrosion resistance of stainless steel" Corrosion Science, vol. 49, pp. 1933-1948 (2007).
- Elemental Charts from [chemicalelements.com](http://chemicalelements.com); retrieved Jul. 27, 2017.
- Song et al., "Corrosion Mechanisms of Magnesium Alloys" Advanced Engg Materials, vol. 1, No. 1 (1999).
- Zhou et al., "Tensile Mechanical Properties and Strengthening Mechanism of Hybrid Carbon Nanotubes . . ." Journal of Nanomaterials, 2012; 2012:851862 (doi: 10.1155/2012/851862) Figs. 6 and 7.
- Trojanova et al., "Mechanical and Acoustic Properties of Magnesium Alloys . . ." Light Metal Alloys Application, Chapter 8, Published Jun. 11, 2014 (doi: 10.5772/57454) p. 163, para. [0008], [0014-0015]; [0041-0043].
- AZoNano "Silicon Carbide Nanoparticles-Properties, Applications" <http://www.amazon.com/articles.aspx?ArticleID=3396> p. 2, Physical Properties, Thermal Properties (May 9, 2013).
- AZoM "Magnesium AZ91D-F Alloy" <http://www.amazon.com/articles.aspx?ArticleID=8670> p. 1, Chemical Composition; p. 2 Physical Properties (Jul. 31, 2013).
- Elasser et al., "Silicon Carbide Benefits and Advantages . . ." Proceedings of the IEEE, 2002; 906(6):969-986 (doi: 10.1109/JPROC.2002.1021562) p. 970, Table 1.
- Lan et al., "Microstructure and Microhardness of SiC Nanoparticles . . ." Materials Science and Engineering A; 386:284-290 (2004).
- Casati et al., "Metal Matrix Composites Reinforced by Nanoparticles", vol. 4:65-83 (2014).
- Hemanth, "Fracture Behavior of Cryogenically solidified aluminum-alloy reinforced with Nano-ZrO<sub>2</sub> Metal Matrix Composites (CNMMCs)", Journal of Chemical Engineering and Materials Science, vol. 2(8), pp. 110-121 (Aug. 2011).
- United States District Court/Northern District of Ohio/Eastern Division, Supplemental Declaration of Dana J. Medlin, Ph.D. in Support of Opposition to Terves LLC'S Motion for Preliminary Injunction in related Case 1:19-CV-1611 (filed Oct. 15, 2020).
- United States District Court/Northern District of Ohio/Eastern Division, Declaration of Andrew Sherman in Support of Terves' Preliminary Injunction Motion in related Case 1:19-CV-1611 (filed May 1, 2020).
- Shimizu et al., "Multi-walled carbon nanotube-reinforced magnesium alloy composites", Scripta Materialia, vol. 58, pp. 267-270 (2008).
- Zhan et al., "Single-wall carbon nanotubes as attractive toughening agents in alumina-based nanocomposites", Nature Materials, vol. 2, pp. 38-42 (Jan. 2003).
- Curtin et al., "CNT-reinforced ceramics and metals", Materials Today, vol. 7, pp. 44-49 (2004).
- Pardo et al., "Corrosion behavior of magnesium/aluminum alloys in 3.5 wt.% NaCl", Corrosion Science, vol. 50, pp. 823-834 (2008).
- Song et L., "Influence of microstructure on the corrosion of diecast AZ91D", Corrosion Science, vol. 41, pp. 249-273 (1999).
- Watarai, "Trend of Research and Development for Magnesium Alloys—Reducing the Weight of Structural Materials in Motor Vehicles", Science & Technology Trends, Quarterly Review, No. 18, pp. 84-97 (Jan. 2006).
- Saravanan et al., "Mechanically Alloyed Carbon Nanotubes (CNT) Reinforced Nanocrystalline AA 4032: Synthesis and Characterization", Journal of Minerals & Materials Characterization & Engineering, vol. 9, No. 11, pp. 1027-1035 (2010).

(56)

## References Cited

## OTHER PUBLICATIONS

- Tsipas et al., "Effect of high energy ball milling on titanium-hydroxyapatite powders", *Powder Metallurgy*, vol. 46, No. 1 pp. 73-77 (2003).
- Xie et al., "TEM Observation of Interfaces between Particles in Al—Mg Powder Compacts Prepared by Pulse Electric Current Sintering", *Materials Transactions*, vol. 43, No. 9, pp. 2177-2180 (2002).
- Elsayed et al., "Effect of Consolidation and Extrusion Temperatures on Tensile Properties of Hot Extruded ZK61 Magnesium Alloy Gas Atomized Powders via Spark Plasma Sintering", *Transactions of JWRI*, vol. 38, No. 2, p. 31.
- Shigematsu et al., "Surface treatment of AZ91D magnesium alloy by aluminum diffusion coating", *Journal of Materials Science Letters*, vol. 19, pp. 473-475 (2000).
- Spencer et al., "Fluidized Bed Polymer Particle ALD Process for Producing HDPE/Alumina Nanocomposites", 12th International Conference on Fluidization, vol. RP4 (2007).
- Maisano, "Cryomilling of Aluminum-Based and Magnesium-Based Metal Powders", Thesis, Virginia Tech (Jan. 2006).
- Walters et al., "A Study of Jets from Unsintered-Powder Metal Lined Nonprecision Small-Caliber Shaped Charges", Army Research Laboratory, Aberdeen Proving Group, MC 21005-5066 (Feb. 2001). National Physical Laboratory, "Bimetallic Corrosion" Crown (C) p. 1-14 (2000).
- Ye et al., "Review of recent studies in magnesium matrix composites", *Journal of Material Science*, vol. 39, pp. 6153-6171 (2004).
- Hassan et al., "Development of a novel magnesium-copper based composite with improved mechanical properties", *Materials Research Bulletin*, vol. 37, pp. 377-389 (2002).
- Ye et al., "Microstructure and tensile properties of Ti6Al4V/AM60B magnesium matrix composite", *Journal of Alloys and Composites*, vol. 402, pp. 162-169 (2005).
- Kumar et al., "Mechanical and Tribological Behavior of Particulate Reinforced Aluminum metal Matrix Composite", *Journal of Minerals & Materials Characterization and Engineering*, vol. 10, pp. 59-91 (2011).
- Majumdar, "Micromechanics of Discontinuously Reinforced MMCs", *Engineering Mechanics and Analysis of Metal-Matrix Composites*, vol. 21, pp. 395-406.
- United States District Court/Northern District of Ohio/Eastern Division, Memorandum Opinion and Order in related Case 1:19-CV-1611 (issued Mar. 29, 2021).
- United States District Court/Northern District of Ohio/Eastern Division, Second Rebuttal Rule 26 Report of Lee A. Swanger, Ph.D., P.E. in related Case 1:19-CV-1611 (filed Nov. 24, 2020).
- U.S. Patent and Trademark Office, Declaration of Dana J. Medlin in Support of Request for Ex Parte Reexamination of U.S. Pat. No. 10,329,653 (filed Jul. 6, 2021).
- Ashby, "Teach Yourself Phase Diagrams and Phase Transformations", Cambridge, 5th Edition, pp. unknown (March 2009).
- Callister, Materials Science and Engineering an Introduction, 6th Edition, New York, pp. unknown (2003).
- Hanson et al. Constitution of Binary Alloys, McGraw-Hill Book Co. Inc., pp. unknown (1958).
- MSE 2090: Introduction to Materials Science, Chapter 9, pp. unknown (date unknown).
- Metals Handbook, "Metallography, Structures and Phase Diagrams", Aluminum-Magnesium, American Society For Metals, 8th Edition, vol. 8, pp. unknown (1973).
- Metals Handbook, "Metallography, Structures and Phase Diagrams", Magnesium-Nickel, American Society for Metals, 8th Edition, vol. 8, pp. unknown (1973).
- Principles and Prevention of Corrosion, "Volts versus saturated calomel reference electrode", D.A. Jones, p. 170 (1996).
- Medlin, "Mass Balance", handwritten notes (Nov. 2020).
- Metals Handbook, "Metallography, Structures and Phase Diagrams", Aluminum-Iron, American Society for Metals, 8th Edition, vol. 8, p. 260 (1973).
- Metals Handbook, "Metallography, Structures and Phase Diagrams", Aluminum-Nickel, American Society for Metals, 8th Edition, vol. 8, p. 261 (1973).
- Metals Handbook, "Metallography, Structures and Phase Diagrams", Aluminum-Copper, American Society for Metals, 8th Edition, vol. 8, p. 259 (1973).
- Metals Handbook, "Metallography, Structures and Phase Diagrams", Silver-Aluminum, American Society for Metals, 8th Edition, vol. 8, p. 252 (1973).
- Medlin, Declaration of Dona J. Medlin Ph.D., P.E., FASM Under 37 CFR Section 1.68 in Support of Petition For Inter Partes Review of U.S. Pat. No. 9,903,010 (Sep. 2020).
- Li, Qiang, "Translation Declaration and Translation of China Patent Publication No. 103343271" (Jun. 2020).
- Ho et al., The mechanical behavior of magnesium alloy AZ91 reinforced with fine copper particulates, *Materials Science and Engineering A369*, pp. 302-308 (2004).
- Trojanova et al., "Mechanical and fracture properties of an AZ91 Magnesium alloy reinforced by Si and SiC particles", *Composites Science and Technology*, vol. 69, pp. 2256-2264 (2009).
- Lin et al., "Formation of Magnesium Metal Matrix Composites Al2O3p/AZ91D and Their Mechanical Properties After Heat Treatment" *Acta Metallurgica Slovaca*, vol. 16, pp. 237-245 (2010).
- Saravanan et al., "Fabrication and characterization of pure magnesium-30 vol. SiCP particle composite", *Material Science and Eng.*, vol. 276, pp. 108-116 (2000).
- Song et al., "Texture evolution and mechanical properties of AZ31B magnesium alloy sheets processed by repeated unidirectional bending", *Journal of Alloys and Compounds*, vol. 489, pp. 475-481 (2010).
- Blawert et al., "Magnesium secondary alloys: Alloy design for magnesium alloys with improved tolerance limits against impurities", *Corrosion Science*, vol. 52, No. 7, pp. 2452-2468 (Jul. 1, 2010).
- Wang et al., "Effect of Ni on microstructures and mechanical properties of AZ1 02 magnesium alloys" *Zhuzao Foundry, Shenyang Zhuzao Yanjusuo*, vol. 62, No. 1, pp. 315-318 (Jan. 1, 2013).
- Kim et al., "Effect of aluminum on the corrosions characteristics of Mg—4Ni—xAl alloys", *Corrosion*, vol. 59, No. 3, pp. 228-237 (Jan. 1, 2003).
- Unsworth et al., "A new magnesium alloy system", *Light Metal Age*, vol. 37, No. 7-8, pp. 29-32 (Jan. 1, 1979).
- Geng et al., "Enhanced age-hardening response of Mg—Zn alloys via Co additions", *Scripta Materialia*, vol. 64, No. 6, pp. 506-509 (Mar. 1, 2011).
- Zhu et al., "Microstructure and mechanical properties of Mg6ZnCuO.6Zr (wt.%) alloys", *Journal of Alloys and Compounds*, vol. 509, No. 8, pp. 3526-3531 (Dec. 22, 2010).
- International Search Authority, International Search Report and Written Opinion for PCT/GB2015/052169 (dated Feb. 17, 2016). Search and Examination Report for GB 1413327.6 (dated Jan. 21, 2015).
- Magnesium Elektron Test Report (Mar. 8, 2005).
- New England Fishery Management Counsel, "Fishery Management Plan for American Lobster Amendment 3" (Jul. 1989).
- Emly, E.F., "Principles of Magnesium Technology" Pergamon Press, Oxford (1966).
- Shaw, "Corrosion Resistance of Magnesium Alloys", *ASM Handbook*, vol. 13A, pp. 692-696 (2003).
- Hanawalt et al., "Corrosion studies of magnesium and its alloys", *Metals Technology*, Technical Paper 1353 (1941).
- The American Foundry Society, Magnesium alloys, casting source directory 8208, available at [www.afsinc.org/files/magnes.pdf](http://www.afsinc.org/files/magnes.pdf).
- Rokhlin, "Magnesium alloys containing rare earth metals structure and properties", *Advances in Metallic Alloys*, vol. 3, Taylor & Francis (2003).
- Ghali, "Corrosion Resistance of Aluminum and Magnesium Alloys" pp. 382-389, Wiley Publishing (2010).
- Kim et al., "High Mechanical Strengths of Mg—Ni—Y and MG—Cu Amorphous Alloys with Significant Supercooled Liquid Region", *Materials Transactions*, vol. 31, No. 11, pp. 929-934 (1990).
- Tekumalla et al., "Mechanical Properties of Magnesium-Rare Earth Alloy Systems", *Metals*, vol. 5, pp. 1-39 (2014).

(56)

**References Cited**

OTHER PUBLICATIONS

- State Intellectual Property Office of People's Republic of China, First Office Action for corresponding China Patent Application No. 201580020103.7 (dated Aug. 11, 2017).
- Terves LLC, Response to First Office Action for China Patent Application No. 201580020103.7 (Official Translation dated Jul. 2, 2020).
- Medlin, Dana, "Expert Report of Dana J. Medlin, PhD, PE, FASM in the Matter of *Terves LLC v. Yueyang Aerospace New Materials Co., Ltd.*, et al.", US District Court for the Northern District Of Ohio, Eastern Division, Case No. 1:19-cv-1661 (Jul. 27, 2021).
- Medlin, Dana, "Expert Rebuttal Report of Dana J. Medlin, PhD, PE, FASM", US District Court for the Northern District of Ohio, Eastern Division, Case No. 1:19-cv-1661 (Aug. 27, 2021).
- Yueyang Aerospace New Materials Co, Ltd, et al., "The Ecometal Defendant's Final Invalidity, Non-Infringement, and Unenforceability Contentions", US District Court for the Northern District of Ohio, Eastern Division, Case No. 1:19-cv-1661 (Jul. 6, 2020).
- Ralston and Birbilis, "Effect of Grain Size on Corrosion: A Review", Corrosion, vol. 66, No. 7, pp. 075005-01 thru 13 (2010).
- Sherman, Andrew, "Declaration of Andrew J. Sherman Under 37 CFR § 1.132" in Ex Parte Reexamination of U.S. Appl. No. 90/014,795 (Jan. 14, 2021).
- Swanger, Lee A., "Declaration of Lee A. Swanger, PhD, PE Under 37 CFR § 1.132" in Ex Parte Reexamination of U.S. Appl. No. 90/014,795 (Jan. 14, 2021).



Figure 1



Figure 2



Figure 3



Figure 4



Figure 5



Figure 6



Figure 7

| Sample         | angle | loss (cc) |
|----------------|-------|-----------|
| TAx-100E       | 30    | 0.1301    |
| TAx-100E       | 60    | 0.1483    |
| TAx-100E       | 90    | 0.0442    |
| Gray Cast Iron | 30    | 0.0112    |
| Gray Cast Iron | 60    | 0.0257    |
| Gray Cast Iron | 90    | 0.0162    |
| TA-MMC170130-1 | 30    | 0.0049    |
| TA-MMC170130-1 | 60    | 0.0380    |
| TA-MMC170130-1 | 90    | 0.0323    |

**Figure 8**

## DEGRADABLE METAL MATRIX COMPOSITE

The present invention is a continuation application of U.S. patent application Ser. No. 16/045,924 filed Jul. 26, 2018, which in turn claims priority on U.S. Provisional Application Ser. No. 62/537,707 filed Jul. 27, 2017, which are incorporated herein by reference.

### TECHNICAL FIELD OF THE INVENTION

The present invention relates to the composition and production of an engineered degradable metal matrix composite that is useful in constructing temporary systems requiring wear resistance, high hardness, and/or high resistance to deformation in water-bearing applications such as, but not limited to, oil and gas completion operations. In particular, the engineered degradable metal matrix composite of the present invention includes a core material and a degradable binder matrix, and which composite includes the following properties: A) repeating ceramic particle core material of 20-90 vol. %, B) degradable metallic binder/matrix, C) galvanically-active phases formed in situ from a melt and/or added as solid particles, D) degradation rate of 5-800 mg/cm<sup>2</sup>/hr., or equivalent surface regression rates of 0.05-5 mm/hr. (and all values and ranges therebetween) in selected fluid environments such as, but not limited to, freshwater, brines and/or fracking liquids at a temperature of 35-200° C., and E) hardness exceeding 22 Rockwell C (ASTM E 18-07). The method of manufacturing the composite in accordance with the present invention includes the preparation of a plurality of ceramic particles, with or without galvanically-active materials such as, but not limited to, iron, nickel, copper, titanium, or cobalt, and infiltrating the ceramic particles with a degradable metal such as, but not limited to, magnesium, aluminum, magnesium alloy or aluminum alloy.

### BACKGROUND OF THE INVENTION

The preparation of magnesium and aluminum degradable metal compositions, as well as degradable polymer compositions, has resulted in rapid commercialization of interventionless tools, including plugs, balls, valves, retainers, centralizers, and other applications. Generally, these products consist of materials that are engineered to dissolve or to corrode. Dissolving polymers and some powder metallurgy metals have been used in the oil and gas recovery industry.

While these prior art degradable systems have enjoyed success in reducing well completion costs, their ability to withstand deformation and to resist erosion in flowing fluid or to embed in steel casing are not suitable for a number of desired applications. For example, in the production of dissolving frac plugs, ceramic or steel inserts are currently used for gripping surfaces (to set the plug into the steel casing). Requirements for these grips include: a hardness higher than the steel casing; mechanical properties, including compression strength, deformation resistance (to retain a sharp edge); and fracture toughness that must be sufficient to withstand the setting operation where they are embedded slightly into the steel casing. Other applications such as 1) pump down seats currently fabricated from grey cast iron need to be milled out, and 2) frac balls or cones having very small overlaps with the seat (1/16" or less) currently have limited pressure ratings with dissolvable materials due to limited swaging or deformation resistance of current materials.

For applications such as seats and valve components and other sealing surfaces that are subjected to sand or proppant flow, existing magnesium, aluminum, or polymer alloy degradables have insufficient hardness and erosion resistance. In frac ball applications, metallic and polymer degradable balls deform, swage, and shear in such conditions, thereby limiting their pressure rating in small overlap (e.g., below 1/8" overlap) applications.

Sintered and cast products of metal matrix ceramic (MMC) plus metallic composites have been used in structural parts, wear parts, semiconductor substrates, printed circuit boards, high hardness and high precision machining materials (such as cutting tools, dies, bearings), and precision sinter molding materials, among other applications. These materials have found particular use in wear and high temperature highly loaded applications such as bearing sleeves, brake rotors, cutting tools, forming dies, and aerospace parts. Generally, these materials are selected from non-reactive components and are designed to not degrade, and the MMC and the cermets are formulated to resist all forms of corrosion/degradation, including wear and dissimilar metal corrosion.

To overcome the limitations of current degradable materials, a new material is required that has high strength, controlled degradation, and high hardness. Ideally, these high hardness degradable components and materials would also be able to be manufactured by a method that is low cost, scalable, and results in a controlled corrosion rate in a composite or alloy with similar or increased strength compared to traditional engineering alloys such as aluminum, magnesium, and iron and with hardnesses higher than cast iron. Ideally, traditional heat treatments, deformation processing and machining techniques could be used without impacting the dissolution rate and reliability of such components.

### SUMMARY OF THE INVENTION

The present invention relates to the composition and production of an engineered degradable metal matrix composite that is useful in constructing temporary systems requiring wear resistance, high hardness, and/or high resistance to deformation in water-bearing applications such as, but not limited to, oil and gas completion operations. In one non-limiting embodiment of the invention, the engineered degradable metal matrix composite includes a core material and a degradable binder matrix, and which composite includes the following properties: A) a repeating ceramic particle core material of 20-90 vol. % (and all values and ranges therebetween), B) a degradable metallic binder/matrix of 10-75 vol. % (and all values and ranges therebetween), C) galvanically-active phases formed in-situ from a melt or added as solid particles, D) a degradation rate being controlled to rates of 5-800 mg/cm<sup>2</sup>/hr. (and all values and ranges therebetween), or equivalent surface regression rates of 0.05-5 mm/hr. (and all values and ranges therebetween) at a temperature of 35-200° C. (and all values and ranges therebetween) in 100-100,000 ppm (and all values and ranges therebetween) water or brines, and E) a hardness exceeding 22 (e.g., 22.01-60 Rockwell C and all values and ranges therebetween). Fluids seen in completion operations and which the composite of the present invention can be used in include 1) freshwater (generally 300-5000 ppm salt content), 2) drilling and completion brines including seawater which are generally chlorides and bromides of potassium, calcium, sodium, cesium, and zinc from about 5000 ppm to as high as 500,000 ppm or more, 3) some formates

and acidic fluids, or 4) fluid produced or flowed back from the well formation which can include chlorides and carbonate salts. As can be appreciated, in some cases special fluids can be run in the well formation to cause or trigger the dissolution of the composite of the present invention, or a salt or chemical pills can be added to the fluid to cause or trigger the dissolution of the composite of the present invention. The present inventions also relates to the method of manufacturing the engineered degradable metal matrix composite of the present invention, which method includes the preparation of a plurality of ceramic particles, with or without galvanically-active materials such as, but not limited to, iron, nickel, copper, titanium, or cobalt, and infiltrating the ceramic particles with a degradable metal such as, but not limited to, magnesium or aluminum alloy.

In one non-limiting aspect of the invention, the invention relates to the formation of high hardness, wear-, deformation-, and erosion-resistant metal matrix composite materials that exhibit controlled degradation rates in aqueous media at temperatures that are at least 35° C., and typically about 35-200° C. (and all values and ranges therebetween) conditions. The ability to control the dissolution of a down hole well component in a variety of solutions is very important to the utilization of interventionless drilling, production, and completion tools such as sleeves, frac balls, hydraulic actuated tooling, scrapers, valves, screens, perforators and penetrators, knives, grips/slips, and the like. Reactive materials useful in this invention that dissolve or corrode when exposed to acid, salt, or other wellbore conditions have been proposed for some time. Incorporated by reference are U.S. Pat. Nos. 9,903,010; 9,757,796, and US Publication No. 2015/0239795 which describe techniques for creating and manufacturing dissolvable magnesium alloys through the addition of galvanically-active phases.

To obtain resistance to one type of degradation such as wear, but also to have high susceptibility to another type of corrosion such as aqueous corrosion, a composite containing two distinct phases was found to be required. One phase, being a high hardness phase, is present in large amounts (greater than 30 vol. %, and typically greater than 50 vol. %) of the composite. This high hardness phase provides resistance to wear and erosion and increases the hardness and deformation resistance of the composite. Useful deformation resistance is achieved by a second ceramic phase present in an amount of at least 10 vol. % in the composite. The deformation resistance can be enhanced by use of a higher aspect ratio ceramic phase. Useful hardness increases in the composite can be achieved with greater than 35% volumetric loading of the second ceramic phase, and can be further increased with increasing the loading. By selecting the right materials and controlling their percentages, distribution, and surface areas, novel composites can be fabricated that resist one type of degradation (namely wear or erosion) but are highly susceptible to other types of degradation (aqueous corrosion).

To achieve the desired degradation, galvanically-active phase(s) are required. This is achieved by adding a second phase either as a separate powder blended with the ceramic powder, a coating on the ceramic particles, and/or in situ by solidification or precipitation for the melt or solid solution. For example, when magnesium is selected as a degradable matrix alloy, the galvanically active phase in the magnesium matrix alloy can be formed of 1) iron and/or carbon (graphite) particle additions or coatings on ceramic particles, and/or 2) through the formation of Mg<sub>2</sub>M (where M is nickel, copper, or cobalt) -active intermetallics created during solidification from a highly alloyed melt. In terms of

effectiveness for increasing corrosion rates, the following ranking can be used: Fe>Ni>Co>Cu, with carbon falling between nickel and copper depending on its structure. In another example, when aluminum or aluminum alloys are selected as the degradable matrix alloy, additions of gallium and/or indium are effective for managing corrosion, and such metals can be added as a coating on the ceramic particles, as intermetallic particles, and/or by adding as a solid solution from an aluminum alloy melt. Additional strengthening phases and solid solution material can be used to accelerate or inhibit corrosion rates. In general, aluminum and magnesium decrease corrosion rates, while zinc is neutral or can enhance corrosion rates. Corrosion rates of 0.02-5 mm/hr. (and all values and ranges therebetween) at a temperature of 35-200° C. for the composite can be achieved in freshwater or brine environments.

When the ceramic content is significant (greater than about 20 vol. %), the ceramic particles begin to block the corrosion process and inhibit the access of the aqueous solution to the degradable metal matrix. A 10-20 times decrease in degradation rates has been observed in a composite that includes 50 vol. % ceramic content. As such, the addition of ceramic content that is greater than about 20 vol. % has been found to result in a non-linear decrease in degradation rates. The decrease is generally more substantial with very fine particles of ceramic material (e.g., less than 100 micron). To compensate for a lower surface area exposed for dissolution due to a large inert loading of ceramic, a much higher dissolution rate in the matrix must be used to generate useful degradation rates. This can be accomplished by substituting more active catalysts (e.g., iron for nickel, nickel for copper), and by reducing the content of inhibiting phases (aluminum or other more cathodic metals). This may be done by moving to a ZK series alloy in magnesium from a WE or AZ series, for example. In general, the degradable matrix alloy and catalyst (galvanically-active phase) is selected to be 5-25 times as active (faster rate) than an equivalent non-composite system.

By selecting the right alloy chemistry and catalyst phase and its content (primarily exposed surface area), degradable MMCs are possible over temperatures ranging from 35-200° C., in low salinity (less than 1000 ppm dissolved solids, and typically 1-5 vol. % dissolved solids, normally KCl, NaCl), and heavy brines (CaCl<sub>2</sub>, CaBr<sub>2</sub>, ZnBr<sub>2</sub>, carbonates, etc.). By reducing galvanically-active phases and adding inhibiting phases, materials having suitable corrosion/degradation rates in acidic media (such as 5 vol. % HCl or formic acid) can also be created.

In summary, the present invention relates to a degradable high hardness composite material that includes 1) plurality of ceramic particles having a hardness greater than 50 HRC and up to 10,000 VHN that forms 20-90 vol. % of the composite, 2) degradable alloy matrix selected from magnesium, aluminum, zinc, or their alloys that forms 10-75 vol. 55 % of the composite, 3) plurality of degradation catalyst particles, zones, and/or regions that are galvanically-active (wherein such particles, zones, and/or regions contain one or more galvanically-active elements such as, but not limited to, iron, nickel, copper, cobalt, silver, gold, gallium, bismuth, lead, carbon or indium metals) and whose content is engineered to control degradation rates of 5-800 mg/cm<sup>2</sup>/hr. (and all values and ranges therebetween), or equivalent surface regression rates of 0.05-5 mm/hr. (and all values and ranges therebetween) at a temperature of 35-200° C. (and all values and ranges therebetween) in 100-100,000 ppm (and all values and ranges therebetween) water or brines, and 4) ceramic particle content is 25-90 vol. % (and all values and

ranges therebetween); to create a composite having a hardness of greater than 22 Rockwell C (ASTM E-18), and typically greater than 30 Rockwell C, and typically up to 70 Rockwell C (and all values and ranges therebetween).

The ceramic or intermetallic particles in the degradable high hardness composite material can be selected from metal carbides, borides, oxides, silicides, or nitrides such as, but not limited to, SiC, B<sub>4</sub>C, TiB<sub>2</sub>, TiC, Al<sub>2</sub>O<sub>3</sub>, MgO, SiC, Si<sub>3</sub>N<sub>4</sub>, ZrO<sub>2</sub>, ZrSiO<sub>4</sub>, SiB<sub>6</sub>, SiAlON, WC, or other high hardness ceramic or intermetallic phases. The particles can be hollow or solid.

The ceramic or intermetallic particles in the degradable high hardness composite material can have a particle size of 0.1-1000 microns (and all values and ranges therebetween), and typically 5-100 microns, and may optionally have a broad or multimodal distribution of sizes to increase ceramic content.

Some or all of the ceramic or intermetallic particles in the degradable high hardness composite material can be shards, fragments, preformed or machined shapes, flakes, or other large particles with dimensions of 0.1-4 mm (and all values and ranges therebetween).

The surface coating on the ceramic or intermetallic particles can include nickel, iron, cobalt, titanium, nickel and/or copper to control dissolution and wetting as well as provide some or all of the galvanic activation. The surface coating on the ceramic or intermetallic particles can include magnesium, zinc, aluminum, tin, titanium, nickel, copper and/or other wetting agent to facilitate melt infiltration and/or particle distribution. The surface coating thickness is generally at least 60 nm and typically up to about 100 microns (and all values and ranges therebetween). The surface coating generally constitutes at least 0.1 wt. % of the coated ceramic or intermetallic particle, and typically constitutes up to 15 wt. % of the coated ceramic or intermetallic particle (and all values and ranges therebetween). The ceramic or intermetallic particles can be coated by a variety of coating techniques (e.g., chemical vapor deposition, wurster coating, physical vapor deposition, hydrometallurgy processes and other chemical or physical methods.

The particle surface of the ceramic or intermetallic particles can be modified with metal particles or other techniques to control the spacing of the ceramic particles, such as through the addition of titanium, zirconium, niobium, vanadium, and/or chromium active metal particles. Generally, these metal particles constitute about 0.1-15 wt. % (and all values and ranges therebetween) of the coated ceramic or intermetallic particles. It has been found that by coating the ceramic or intermetallic particles with such metals prior to adding the matrix metal, the metal coating facilitates in the building of a metal layer on the ceramic or intermetallic particles to create a boundary between the ceramic or intermetallic particles in the final composite, thereby effectively separating the ceramic or intermetallic particles in the final composite by at least 1.2 and typically at least 2× the coating thickness of the metal coating on the ceramic or intermetallic particles that exist on the ceramic or intermetallic particles prior to the addition of the matrix metal.

The degradable alloy matrix includes magnesium, aluminum, zinc, and their combinations and alloys which forms 10-75 vol. % of the composite, and the composite may optionally contain one or more active metals such as calcium, barium, indium, gallium, lithium, sodium, or potassium. Such active metals, when used, constitute about 0.05-10 wt. % (and all values and ranges therebetween) of the metal matrix material.

The degradation rate of the degradable high hardness composite material can be 0.01-5 mm/hr. (and all values and ranges therebetween) in fresh water or brines at a temperature of 35-200° C. (and all values and ranges therebetween).

5 The degradation rate of the degradable high hardness composite material can be engineered to be 0.05-5 mm/hr. (and all values and ranges therebetween) in a selected brine composition with a total dissolved solids of 300-300,000 ppm (and all values and ranges therebetween) of chloride, bromide, formate, or carbonate brines at selected temperatures of 35-200° C. (and all values and ranges therebetween).

10 The degradable high hardness composite material can have a compression strength of greater than 40 ksi, and typically greater than 80 ksi, and more typically greater than 100 ksi.

15 The degradable high hardness composite material can be fabricated by powder metallurgy, melt infiltration, squeeze casting, or other metallurgical process to create a greater than 92% pore-free structure, and typically greater than 98% pore-free structure.

20 The degradable high hardness composite material can be deformed and/or heat treated to develop improved mechanical properties, reduce porosity, or to form net shape or near net shape dimensions.

25 The degradable high hardness composite material can be useful in oil and gas or other subterranean operations, including a seat, seal, ball, sleeve, grip, slip, valve, valve component, spring, retainer, scraper, poppet, penetrator, perforator, shear, blade, insert, or other component requiring wear, erosion, or deformation resistance, edge retention, or high hardness.

30 The degradable high hardness composite material can be used as a portion of a component or structure, such as a surface coating or cladding, an insert, sleeve, ring, or other limited volume portion of a component or system

35 The degradable high hardness composite material can be applied to a component surface through a cold spray, thermal spray, or plasma spray process

40 The degradable high hardness composite material can be fabricated using pressure-assisted or pressureless infiltration of a bed of ceramic particles, wherein the galvanic catalyst, dopant, or phase is formed in situ (from solidification and precipitation of the melt), ex situ (from addition of particles or coatings in the powder bed or preform) sources, and/or formed in situ prior to or during infiltration or composite preparation.

45 The degradable high hardness composite material can be fabricated through powder metallurgy processes, including mixing of powders, compacting, and sintering, or alternate isostatic pressing, spark plasma sintering, powder forging, injection molding, or similar processes to produce the desired composite.

50 The degradable high hardness composite material can have a ceramic phase that contains flakes, platelets, whiskers, or short fibers with an aspect ratio of at least 4:1, and typically 10:1 or more.

55 These and other advantages of the present invention will become more apparent to those skilled in the art from a review of the figures and the description of the embodiments and claims.

#### BRIEF DESCRIPTION OF FIGURES

60 FIGS. 1-3 illustrate various non-limiting degradable metal matrix composite structures in accordance with the present invention. These figures illustrate the ceramic particles dis-

persed into a dissolvable metal matrix, generally at a concentration of 30-60 vol. %. FIG. 1 illustrates a composite formed of ceramic particles 12 in a dissolvable metallic matrix 10. FIG. 2 illustrates a composite formed of ceramic particles 16 in a water degradable matrix 14 with the entire composite surrounded by a protective coating 18 (e.g., degradable polymer material, degradable metal) wherein the coating is triggered to degrade or is removed by some method. FIG. 3 illustrates a composite formed of degradable matrix 20 with ceramic particles 22 and platelet or fiber mechanically reinforcement from flakes, platelets, or fibers 24.

FIG. 4 is a chart illustrating the galvanic series showing electronegative materials. Magnesium is a very electronegative material and undergoes active corrosion when coupled with a variety of metals. Particularly effective are iron, nickel, copper, and cobalt, as well as  $\text{Fe}_3\text{Al}$  since they do not form insulating oxides under typical conditions and, as such, maintain electrical connectivity with the fluid. Dissolution rates are controlled by the amount and size of these additives, driven by the electrically connected surface area of the positive and negative metals in the galvanic series.

FIGS. 5 and 6 illustrate a representative microstructure for a magnesium-graphite composite that is galvanically active and could be used as a low friction or deformation-resistant structure, but is not generally effective for wear resistance. FIG. 5 is a magnesium-coated graphite, consolidated magnesium-germanium part, and microstructure of  $\text{Mg}_2\text{B}_4\text{C}$  MMC. FIG. 6 is a magnesium-iron-germanium reactive MMC composite microstructure.

FIG. 7 illustrates the comparative impingement loss at 30° impact angle of a typical seat versus material. FIG. 7 also illustrates the improvement in erosion resistance of a degradable Mg— $\text{B}_4\text{C}$  composition of the present invention (Tervalloy™ MMC with 149 micron D50 ceramic particles) as compared to the baseline cast iron materials used today, and also to a non-MMC degradable magnesium alloy.

FIG. 8 is a table that illustrates impingement erosion loss of dissolvable alloys, hardened grey cast iron, and dissolvable magnesium metal matrix composite at different impingement angles.

#### DETAILED DESCRIPTION OF NON-LIMITING EMBODIMENTS OF THE INVENTION

The present invention relates to the composition and production of an engineered degradable metal matrix composite that is useful in constructing temporary systems requiring wear resistance, high hardness, and/or high resistance to deformation in water-bearing applications such as, but not limited to, oil and gas completion operations. In one non-limiting embodiment of the invention, the engineered degradable metal matrix composite includes a core material and a degradable binder matrix, and which composite includes the following properties: A) repeating ceramic particle core material of 20-90 vol. % of the composite; B) degradable metallic binder/matrix of 10-75 vol. % of the composite; C) galvanically-active phases formed in situ from a melt and/or added as solid particles that form 0.03-10 vol. % (and all values and ranges therebetween) of the composite; D) degradation rate being controlled to 0.1-5 mm/hr. in selected fluid environments including freshwater and brines at 35-200° C.; and E) hardness of the composite that exceeds 25 Rockwell C. The present inventions also relates to the method of manufacturing the engineered degradable metal matrix composite, which method includes the preparation of a plurality of ceramic particles, with or

without galvanically-active materials such as, but not limited to, iron, nickel, copper, or cobalt, and infiltrating the ceramic particles with a degradable metal such as, but not limited to, magnesium or aluminum alloy. The invention 5 also relates to the formation of high hardness, wear-, deformation-, and erosion-resistant metal matrix composite materials that exhibit controlled degradation rates in aqueous media at a temperature of at least 35° C., and typically about 10 35-200° C. (and all values and ranges therebetween) conditions. The ability to control the dissolution of a down hole 15 well component in a variety of solutions is very important to the utilization of interventionless drilling, production, and completion tools such as sleeves, frac balls, hydraulic actuated tooling, scrapers, valves, screens, perforators and penetrators, knives, grips/slips, and the like.

The invention combines corrodible materials that include 20 highly electronegative metals of magnesium, zinc, and/or aluminum, combined with a high hardness, generally inert phase such as SiC,  $\text{B}_4\text{C}$ , WC,  $\text{TiB}_2$ ,  $\text{Si}_3\text{N}_4$ , TiC,  $\text{Al}_2\text{O}_3$ ,  $\text{ZrO}_2$ , 25 high carbon ferrochrome,  $\text{Cr}_2\text{O}_3$ , chrome carbide, or other high hardness ceramic, and a more electropositive, conductive phase generally selected from copper, nickel, iron, silver, lead, gallium, indium, tin, titanium, and/or carbon and 30 their alloys or compounds. Tool steel, hard amorphous or semi-amorphous steel, and/or stellite alloy-type shards, shavings or particles can offer both galvanic and wear 35 resistance. Other electronegative and electropositive combinations can be envisioned, but are generally less attractive due to cost or toxicity. The more electropositive phase should be able to sustain current, e.g., it should be conductive to drive the galvanic current. The ceramic phase is generally dispersed particles which are fine enough to be able to be easily removed by fluid flow and to not plug devices or form restrictions in a wellbore. It is generally accepted that particles having a size that is less than  $\frac{1}{8}$ " are 40 sufficient for this purpose, although most composites of the present invention utilize much finer particles, generally in the 100 mesh, and very often 200 or 325 mesh sizes, down to 2500 mesh (5 micron and below for increase hardness).

The ceramic or intermetallic, high hardness particles are 45 dispersed in an electronegative metal or metal alloy matrix at concentrations at least 25 vol. %, and typically greater than 50 vol. % of the composite. Very high compressive strength and hardness can be achieved when sufficient ceramic volume has been obtained to limit the effects of the 50 electropositive metal matrix on mechanical properties. This property can be obtained at lower ceramic content when using high aspect ratio particles, such as whiskers, flakes, platelets, or fibers, and substantial deformation resistance can be obtained with higher aspect ratio particles.

Because the generally inert ceramic phase (inert primarily 55 due to low conductivity) inhibits corrosion rates, higher corrosion rate electronegative-electropositive alloy couples are generally used. For example, in a magnesium system, 60 eliminating the addition of aluminum from the alloy (to make the matrix more electronegative), or shifting from copper additions to nickel or even iron (with carbon) additions can be used to increase corrosion rates. For example, using a freshwater or low temperature combination metal matrix (such as Terves FW) instead of a higher temperature brine dissolvable (such as TervAlloy™ TAX-100E and TAX-50E) can be used to sufficiently boost the corrosion rate of a 65 50 vol. %  $\text{B}_4\text{C}$ —Mg containing composite to reach 35 mg/cm<sup>2</sup>/hr. at 70-90° C. The addition of carbonyl iron particles to the magnesium alloy matrix can be used to form a useful lower temperature brine, or freshwater dissolvable metal matrix composite. Terves FW, TervAlloy™ TAX-100E

and TAX-50E are magnesium or magnesium alloys with 0.05-5 wt. % nickel, and/or 0.5-10 wt. % copper additions. In one non-limiting embodiment, magnesium alloy includes over 50 wt. % magnesium and one or more metals selected from the group consisting of aluminum, boron, bismuth, zinc, zirconium, and manganese, and optionally 0.05-35 wt. % nickel, copper and/or cobalt. In another non-limiting embodiment, the magnesium alloy includes over 50 wt. % magnesium and one or more metals selected from the group consisting of aluminum in an amount of about 0.5-10 wt. %, zinc in amount of about 0.1-6 wt. %, zirconium in an amount of about 0.01-3 wt. %, manganese in an amount of about 0.15-2 wt. %; boron in amount of about 0.0002-0.04 wt. %, and bismuth in amount of about 0.4-0.7 wt. % nickel, copper and/or cobalt. In another non-limiting embodiment, the magnesium alloy includes over 50 wt. % magnesium and one or more metals selected from the group consisting of aluminum in an amount of about 0.5-10 wt. %, zinc in amount of about 0.1-3 wt. %, zirconium in an amount of about 0.01-1 wt. %, manganese in an amount of about 0.15-2 wt. %; boron in amount of about 0.0002-0.04 wt. %, and bismuth in amount of about 0.4-0.7 wt. %, and optionally 0.05-35 wt. % nickel, copper and/or cobalt. In another non-limiting embodiment, the magnesium alloy comprises at least 85 wt. % magnesium; one or more metals selected from the group consisting of 0.5-10 wt. % aluminum, 0.05-6 wt. % zinc, 0.01-3 wt. % zirconium, and 0.15-2 wt. % manganese; and optionally about 0.05-45 wt. % of a secondary metal selected from the group consisting of copper, nickel, cobalt, titanium and iron. In another non-limiting embodiment, the magnesium alloy composite comprises 60-95 wt. % magnesium; 0.01-1 wt. % zirconium; and optionally about 0.05-45 wt. % copper, nickel, cobalt, titanium and/or iron. In another non-limiting embodiment, the magnesium alloy comprises 60-95 wt. % magnesium; 0.5-10 wt. % aluminum; 0.05-6 wt. % zinc; 0.15-2 wt. % manganese; and optionally about 0.05-45 wt. % of copper, nickel, cobalt, titanium and/or iron. In another non-limiting embodiment, the magnesium alloy comprising 60-95 wt. % magnesium; 0.05-6 wt. % zinc; 0.01-1 wt. % zirconium; and optionally about 0.05-45 wt. % of copper, nickel, cobalt, titanium and/or iron. In another non-limiting embodiment, the magnesium alloy comprises over 50 wt. % magnesium; one or more metals selected from the group consisting of 0.5-10 wt. % aluminum, 0.1-2 wt. % zinc, 0.01-1 wt. % zirconium, and 0.15-2 wt. % manganese; and optionally about 0.05-45 wt. % of copper, nickel and/or cobalt. In another non-limiting embodiment, the magnesium alloy comprises over 50 wt. % magnesium; one or more metals selected from the group consisting of 0.1-3 wt. % zinc, 0.01-1 wt. % zirconium, 0.05-1 wt. % manganese, 0.0002-0.04 wt. % boron and 0.4-0.7 wt. % bismuth; and optionally about 0.05-45 wt. % of copper, nickel, and/or cobalt. In another non-limiting embodiment, the magnesium alloy comprises 60-95 wt. % magnesium and 0.01-1 wt. % zirconium. In another non-limiting embodiment, the magnesium alloy comprises over 50 wt. % magnesium and one or more metals selected from the group consisting of aluminum in an amount of about 0.5-10 wt. %, zinc in amount of about 0.1-3 wt. %, zirconium in an amount of about 0.01-1 wt. %, manganese in an amount of about 0.15-2 wt. %, boron in amount of about 0.0002-0.04 wt. %, and bismuth in amount of about 0.4-0.7 wt. %.

The electropositive driving phase can be added by adding soluble or insoluble electropositive particles to the ceramic powder prior to melt infiltration or mixing into a melt by adding the electropositive material as a coating or cladding

to the inert ceramic phase, or by adding as an alloying element that forms a fully liquid phase with the electropositive metal or alloy. In the liquid phase, generally an electropositive metal that forms a eutectic with the electronegative metal and an intermetallic of the electropositive metal can be used. Non-limiting examples of such coatings or claddings are Mg—Ni, Mg—Cu, Mg—Co, and Mg—Ag. FIG. 4 is a chart illustrating the galvanic series showing electronegative materials (magnesium through cadmium, electronegative being more electronegative than steel), and electropositive metals (steel through carbon).

The electropositive driving phase can also be added to electropositive metal powders, along with the ceramic phase, and the dissolvable MMC fabricated from powder metallurgy or spray consolidation techniques such as press and sinter, hot isostatic pressing, spark plasma sintering, powder sinter-forging, direct powder extrusion, thermal spray, cold spray, plasma spray, or other powder consolidation techniques.

For melt infiltration of a ceramic preform or powder bed, techniques that can be used include pressureless infiltration (when the ceramic and electronegative metal wet each other, or when the ceramic has been coated with a wetting phase such as a eutectic forming or other easily wet metal), or pressure-assisted infiltration technique such as squeeze casting, high pressure die casting (into the ceramic preform), vacuum casting, or pressure-assisted casting techniques, among others. Particularly at lower ceramic volumes (25-50 vol. %), the particles can be stir-cast, thixocast, or slurry cast by mixing the ceramic (and electropositive material, if in powder form) and formed in the liquid plus ceramic or semi-solid state. Net shape or near net shape fabrication techniques are preferred due to machining cost of precision grinding of the high hardness materials. Active wetting metals such as titanium, zirconium, vanadium, niobium, silicon, boron, and palladium can be added to the melt system to enhance wetting. Surface wetting coatings, often eutectic liquid formers such as niobium, zirconium, magnesium, aluminum, silicon, and/or bismuth can provide strong wetting ability to enhance pressureless infiltration.

After consolidation, the compact can be further formed by forging, extrusion, or rolling. The compact can also be taken back to an elevated temperature, normally in the semi-solid region between the electropositive alloy liquidus and solidus, and formed using closed die forming, squeeze casting, thixocasting, or other semi-solid forming technique.

The cast or formed part can be machined to close tolerances using grinding or electrode discharge machining (EDM). Diamond, CBN, and other high hardness tools can also be used.

The degradable metal matrix composite can be applied as a coating, such as by cold spray, to a separate part, to impart wear-, erosion-, or deformation-resistance, or to slow initial dissolution rates to give added life. A higher degradation rate core is generally desired. In one embodiment, the MMC can be created by surface alloying the higher degradation rate, or lower hardness core, with the ceramic phase by such techniques as friction stir surfacing, supersonic particle spray, or reactive heat treatments (such as boronizing). Other routes to a dual structured component include overcasting or overmolding, or physical assembly with or without an adhesive or bonding step such as forging, hot pressing, friction welding, or use of adhesives.

After machining, parts may be further coated or modified to control initiation of dissolution or to further increase hardness or ceramic content. Techniques such as cold spray, thermal spray, friction surfacing, powder coating, anodizing,

## 11

painting, dip coating, e-coating, etc. may be used to add a surface coating or otherwise modify the surface.

The degradable MMCs of the present invention are particularly useful in the construction of downhole tools for oil and gas, geothermal, and in situ resource extraction applications. The higher hardness enables tools such as reamers, valve seats, ball seats, and grips to be engineered to be fully degradable, eliminating debris as well as the need to retrieve or drill-out the tools. The degradable MMC is a useful, degradable substitute for hardened cast iron in applications such as plug seats and gripping devices for bridge and frac plugs. The degradable MMC is also useful for the design and production of cement plugs, reamers, scrapers, and other devices.

The deformation resistance of the degradable MMCs allows the construction of higher pressure rating valve and plug systems than non-MMC degradable products. For example, a degradable MMC frac ball can withstand 15,000 psi across a  $1/16$ " seat overlap compared to less than 7,000 psi for a conventional degradable magnesium alloy or polymer ball.

FIGS. 1-3 illustrate various degradable metal matrix composite structures in accordance with the present invention. FIGS. 1-3 illustrate a composite formed of ceramic particles 12 in a dissolvable metallic matrix 10.

The composite material is formed by 1) providing ceramic particles, 2) providing a galvanically-active material such as iron, nickel, copper, titanium, and/or cobalt, 3) combining the ceramic particles and galvanically-active material with molten matrix material such as molten magnesium, molten aluminum, molten magnesium alloy or molten aluminum alloy, and 4) cooling the mixture to form the composite material. The cooled and solid dissolvable metallic matrix generally includes over 50 wt. % magnesium or aluminum. The ceramic material is generally coated with the galvanically-active material prior to adding the molten matrix material; however, this is not required.

The galvanically-active material coating on the ceramic material, when precoated, can be applied by any number of techniques (e.g., vapor deposition, dipping in molten metal, spray coating, dry coated and then heated, sintering, melt coating technique, etc.). Generally, each of the coated ceramic particles are formed of 30-98 wt. % ceramic material (and all values and ranges therebetween), and typically greater than 50 wt. % ceramic material. The thickness of the galvanically-active material coating is generally less than 1 mm, and typically less than 0.5 mm.

After the composite is formed, the ceramic material constitutes about 10-85 wt. % (and all values and ranges therebetween) of the composite, the galvanically-active material constitutes about 0.5-30 wt. % (and all values and ranges therebetween) of the composite, and the molten matrix material constitutes about 10-85 wt. % (and all values and ranges therebetween) of the composite.

The dissolution rate of the composite is at least 5-800 mg/cm<sup>2</sup>/hr., or equivalent surface regression rates of 0.05-5 mm/hr. at a temperature of 35-200° C. in 100-100,000 ppm water or brines, and typically at least 45 mg/cm<sup>2</sup>/hr. in 3 wt. % KCl water mixture at 90° C., more typically up to 325 mg/cm<sup>2</sup>/hr. in 3 wt. % KCl water mixture at 90° C.

FIG. 2 illustrates the composite surrounded by a protective coating 18 (e.g., degradable polymer material, degradable metal). The protective coating can be formulated to dissolve or degrade when exposed to one or more activation or trigger conditions such as, but not limited to, temperature, electromagnetic waves, sound waves, certain chemicals, vibrations, salt content, electrolyte content, magnetism,

## 12

pressure, electricity, and/or pH. Once the protective coating has sufficiently dissolved or degraded, the composite is then exposed to the surrounding fluid, thus causing the composite to dissolve, corrode, etc. when exposed to certain surrounding conditions. The protective coating can be formed of one or more metal and/or polymer layers. Non-limiting polymer protective coatings that can be used include ethylene- $\alpha$ -olefin copolymer; linear styrene-isoprene-styrene copolymer; ethylene-butadiene copolymer; styrene-butadiene-styrene copolymer; copolymer having styrene endblocks and ethylene-butadiene or ethylene-butene midblocks; copolymer of ethylene and alpha olefin; ethylene-octene copolymer; ethylene-hexene copolymer; ethylene-butene copolymer; ethylene-pentene copolymer; ethylene-butene copolymer; polyvinyl alcohol (PVA); silicone, and/or polyvinyl butyral (PVB). The thickness of the protective coating is generally less than 3 mm, and more typically about 0.0001-1 mm.

FIG. 3 illustrates a composite formed of degradable matrix 20 with ceramic particles 22 and platelet or fiber mechanically-reinforced flakes, platelets, or fibers 24. The platelets or fibers typically have an aspect ratio of at least 4:1, and typically 10:1 or more. The length of the platelets or fibers is generally less than 3 mm, and typically less than 2 mm. The platelets or fibers, when used, are generally formed of boron carbide silicon carbide, and/or graphite; however, other materials can be used.

## EXAMPLES

In one embodiment, the reactivity of an electrolytically activated reactive composite of magnesium or zinc and iron with ceramic reinforcements is controlled to produce a dissolution rate of 1-10 mm/day (and all values and ranges therebetween), or 0.5-800 mg/cm<sup>2</sup>/hr. (and all values and ranges therebetween) (depending on density) by controlling the relative phase amounts and interfacial surface area of the two galvanically-active phases. In one example, a mechanical mixture of iron or graphite and magnesium is prepared by mechanical milling of magnesium or magnesium alloy powder and 40 vol. % of 30-200 micron iron graphite (and all values and ranges therebetween) graphite or 10 wt. % nickel-coated graphite particles, followed by consolidation using spark plasma sintering or powder forging at a temperature below the magnesium or zinc melting point. The resultant structure has an accelerated rate of reaction due to the high exposed surface area of the iron or graphite cathode phase, but low relative area of the anodic (zinc or magnesium) reactive binder.

The degradable MMC can be used for powder metallurgical processing. FIGS. 5 and 6 illustrate a representative microstructure for a magnesium-graphite composite.

In general, larger ceramic particles, typically above 40 mesh, including flake, impart great impingement erosion resistance at higher angles, while smaller particles, typically below 200 mesh, provide higher sliding wear resistance. Larger particles can also facilitate gripping (in frac plug grips/slips, to facilitate locking a device to a mating surface), such as when mm-sized crushed carbides are added to a dissolvable matrix. Such embedded metal matrix composites can also be used in reamer-type applications as abrasives, such as by adding larger chunks or even preformed shapes, such as crushed, machined, or formed carbides or tool steel discreet elements.

## Example 1

Boron carbide powder with an average particle size of 325 mesh is surface modified by the addition of zinc by blending

## 13

200 grams of B<sub>4</sub>C powder with 15 grams of zinc powder and heated in a sealed, evacuated container to 700° C. to distribute the zinc to the particle surfaces. The zinc-coated B<sub>4</sub>C powder is placed into a graphite crucible and heated to 500° C. with an inert gas cover. In a separate steel crucible, 500 grams of Terves FW low temperature dissolvable degradable magnesium alloy is melted to a temperature of 720° C. The degradable magnesium alloy is poured into the 8-inch deep graphite crucible containing the zinc-coated B<sub>4</sub>C particles sufficient to cover the particles by at least two inches and allowed to solidify.

The material had a hardness 52 Rockwell C, and a measured dissolution rate of 35 mg/cm<sup>2</sup>/hr. in 3 vol. % KCl at 90° C.

## Example 2

300 g of 600 mesh boron carbide powder was placed to a depth of 4"×2" diameter by ten-inch deep graphite crucible containing a two inch layer of 1/4" steel balls (600 g of steel) covered by a 325 mesh steel screen and heated to 500° C. under inert gas. The graphite crucible was heated inside of a steel tube, which was heated with the crucible. Five pounds of Terves FW degradable magnesium alloy were melted in a steel crucible to a temperature of 730° C. and poured into the graphite crucible sufficient to cover the B<sub>4</sub>C and steel balls to reach within two inches of the top of the graphite crucible. The crucible was removed from the furnace and transferred to a 12-ton carver press, where a die was rammed into the crucible forcing the magnesium into and through the powder bed. The crucible was removed from the press and allowed to cool.

The MMC section was separated from the non-MMC material and showed a dissolution rate of 45 gm/cm<sup>2</sup>/hr. at 90° C. in 3 vol. % KCl solution. The measured hardness was 32 Rockwell C.

## Example 3

125 grams of 325 mesh B<sub>4</sub>C powder was blended with 4 grams of 100 mesh titanium powder and sintered at 500° C. to form a rigid preform. A 500 gram ingot of TAx-50E dissolvable metal alloy was placed on top of the preform in a graphite crucible. The crucible was placed in the inert gas furnace and heated to 850° C. for 90 minutes to allow for infiltration of the preform. The infiltrated preform had a hardness of 24 Rockwell C.

## Example 4

Degradable MMC from Example 3 was machined into a frac ball. A 3" ball (3.000+/-0.002), when tested against a cast iron seat with a 45° seat angle and inner diameter of 2.896", was shown to hold greater than 15,000 psig pressure at room temperature. The degradable magnesium frac ball was machined from a high dissolution rate dissolving alloy having a dissolution rate of greater than 100 mg/cm<sup>2</sup>/hr. at 90° C. The frac ball was undermachined by 0.010", to 2.980+/-0.002, and the degradable MMC was applied using cold spray application from a powder generated by ball milling 400 grams of standard degradable alloy machine chips with 600 grams 325 mesh of B<sub>4</sub>C powder using a centerline Windsor SST cold spray system and nitrogen gas as the carrier gas. The ball was then machined to 3"+/-0.002". The ball held >10,000 psig against a 45° cast iron seat at 2.875" inner diameter. The frac ball was designed to

## 14

give two hours of operating time, before dissolving rapidly in less than 48 hours at 90° C. in 3% KCl brine solution.

## Example 5

5 Degradable MMC from Example 3 was machined into a frac ball except that TAx-100E was used instead of TAx-50E. The TAx-100E included trace amounts of iron to form a composite having a hardness of 74HRB and a dissolution rate of 34 mg/cm<sup>2</sup>/hr. in 3% vol. % KCl at 90° C. during a 10 six-hour test. 125 grams of 325 mesh B<sub>4</sub>C powder was blended with 4 grams of 100 mesh titanium powder and sintered at 500° C. to form a rigid preform. A 500 gram ingot of TAx-100E with 0.1% iron was placed on top of the 15 preform in a steel crucible. The crucible was placed in the inert gas furnace and heated to 850° C. for 90 minutes to allow for infiltration of the preform. The infiltrated preform had a hardness of 74HRB and a dissolution rate of 34 20 mg/cm<sup>2</sup>/hr. in 3% KCl at 90° C. during six hours of brine exposure.

It will thus be seen that the objects set forth above, among those made apparent from the preceding description, are 25 efficiently attained, and since certain changes may be made in the constructions set forth without departing from the spirit and scope of the invention, it is intended that all matter contained in the above description and shown in the accompanying drawings shall be interpreted as illustrative and not in a limiting sense. The invention has been described with 30 reference to preferred and alternate embodiments. Modifications and alterations will become apparent to those skilled in the art upon reading and understanding the detailed discussion of the invention provided herein. This invention is intended to include all such modifications and alterations 35 insofar as they come within the scope of the present invention. It is also to be understood that the following claims are 40 intended to cover all of the generic and specific features of the invention herein described and all statements of the scope of the invention, which, as a matter of language, might be said to fall there between. The invention has been described with reference to the preferred embodiments. These and other modifications of the preferred embodiments 45 as well as other embodiments of the invention will be obvious from the disclosure herein, whereby the foregoing descriptive matter is to be interpreted merely as illustrative of the invention and not as a limitation. It is intended to include all such modifications and alterations insofar as they come within the scope of the appended claims.

## What is claimed:

- 50 1. A method for forming a degradable composite, said method comprises:  
 a. providing ceramic particles, a plurality of said ceramic particles having a hardness of greater than 50 HRC;  
 b. providing one or more galvanically-active elements selected from the group consisting of iron, carbon, 55 nickel, copper, cobalt, gallium, indium, and titanium;  
 c. combining ceramic particles and said one or more galvanically-active elements with a degradable metal material, said degradable metal material selected from magnesium, magnesium alloy including greater than 50 wt. % magnesium, and an aluminum alloy;  
 d. dispersing said plurality of ceramic particles and said one or more galvanically-active elements in said degradable metal material while said degradable metal material is in a molten state to form a mixture; and,  
 e. cooling said mixture to form said degradable composite, said degradable composite having a degradation 60 65 70 75 80 85 90 95

**15**

rate of at least 5 mg/cm<sup>2</sup>/hr. in freshwater or brine at a temperature of at least 90° C.

2. The method as defined in claim 1, wherein said degradable composite has a hardness of greater than 22 Rockwell C.

3. The method as defined in claim 1, wherein said degradable composite includes at least 10 vol. % degradable metal material, at least 0.03 vol. % galvanically-active elements, and at least 10 vol. % ceramic particles.

4. The method as defined in claim 1, wherein said degradable composite includes one or more metals selected from the group consisting of calcium, barium, lithium, sodium, potassium, silver, gold, bismuth, lead, and palladium.

5. The method as defined in claim 1, wherein said ceramic particles include one or more materials selected from the group consisting of B<sub>4</sub>C, TiB<sub>2</sub>, TiC, Al<sub>2</sub>O<sub>3</sub>, MgO, SiC, Si<sub>3</sub>N<sub>4</sub>, ZrO<sub>2</sub>, ZrSiO<sub>4</sub>, SiB<sub>6</sub>, SiAlON, WC, carbon ferro-chrome, Cr<sub>2</sub>O<sub>3</sub>, and chrome carbide.

6. The method as defined in claim 1, wherein a plurality of said ceramic particles are surface coated with said one or more galvanically-active elements to form a coating on said ceramic particles prior to being combined with said degradable metal material.

7. The method as defined in claim 1, wherein said coating on said ceramic particles has a thickness of 60 nm to 100 microns.

8. The method as defined in claim 1, wherein said degradable metal material is a magnesium alloy, said magnesium alloy including one or more metal additives selected from the group consisting of nickel, copper, aluminum, boron, bismuth, zinc, zirconium, cobalt, manganese, titanium, and iron.

**16**

9. The method as defined in claim 1, wherein said method further includes the step of coating said degradable composite with a protective coating, said protective coating having a thickness less than 3 mm, said protective coating including a polymer layer.

10. The method as defined in claim 1, wherein said method further includes the step of adding flakes, fibers, or platelets to said mixture of said molten degradable metal matrix, said ceramic or intermetallic particles, and said galvanically-active elements, said flakes, fibers, or platelets having an aspect ratio of at least 4:1, said flakes, fibers, or platelets having a length of up to 4 mm, said flakes, fibers, or platelets including one or more materials selected from the group consisting of boron carbide, silicon carbide, and graphite.

11. The method as defined in claim 9, wherein said method further includes the step of forming said degradable composite to partially or fully form a structure selected from the group consisting of a seat, a seal, a ball, a frac ball, a cone, a wedge, an insert for a slip, a sleeve, a valve, a frac seat, a grip, a slip, a valve component, a spring, a retainer, a scraper, a poppet, a penetrator, a perforator, a shear, a blade, and an insert.

12. The method as defined in claim 9, wherein said ceramic particles have a particle size of 0.1 microns to 1000 microns.

13. The method as defined in claim 9, wherein said degradable composite has a structure that is greater than 92% pore-free.

\* \* \* \* \*